



US012146115B2

(12) **United States Patent**  
**Garellick**

(10) Patent No.: US 12,146,115 B2  
(45) Date of Patent: Nov. 19, 2024

- |      |                                                                                                                                                                                                                                                                                                                                                                                             |                   |         |                                                                                                                                                                                                                                                                                                                                                                                                           |
|------|---------------------------------------------------------------------------------------------------------------------------------------------------------------------------------------------------------------------------------------------------------------------------------------------------------------------------------------------------------------------------------------------|-------------------|---------|-----------------------------------------------------------------------------------------------------------------------------------------------------------------------------------------------------------------------------------------------------------------------------------------------------------------------------------------------------------------------------------------------------------|
| (54) | <b>LOW ASH LUBRICATING COMPOSITIONS FOR CONTROLLING STEEL CORROSION</b>                                                                                                                                                                                                                                                                                                                     | 4,036,771 A       | 7/1977  | Denis et al.                                                                                                                                                                                                                                                                                                                                                                                              |
| (71) | Applicant: <b>Afton Chemical Corporation</b> , Richmond, VA (US)                                                                                                                                                                                                                                                                                                                            | 4,118,329 A       | 10/1978 | Hotten                                                                                                                                                                                                                                                                                                                                                                                                    |
| (72) | Inventor: <b>Kenneth Garelick</b> , Mechanicsville, VA (US)                                                                                                                                                                                                                                                                                                                                 | 4,234,435 A       | 11/1980 | Meinhardt et al.                                                                                                                                                                                                                                                                                                                                                                                          |
| (73) | Assignee: <b>Afton Chemical Corporation</b> , Richmond, VA (US)                                                                                                                                                                                                                                                                                                                             | 4,282,392 A       | 8/1981  | Cupples et al.                                                                                                                                                                                                                                                                                                                                                                                            |
| (*)  | Notice: Subject to any disclaimer, the term of this patent is extended or adjusted under 35 U.S.C. 154(b) by 0 days.                                                                                                                                                                                                                                                                        | 4,537,696 A       | 8/1985  | Beimesch                                                                                                                                                                                                                                                                                                                                                                                                  |
| (21) | Appl. No.: <b>18/068,795</b>                                                                                                                                                                                                                                                                                                                                                                | 4,587,368 A       | 5/1986  | Pratt                                                                                                                                                                                                                                                                                                                                                                                                     |
| (22) | Filed: <b>Dec. 20, 2022</b>                                                                                                                                                                                                                                                                                                                                                                 | 4,747,971 A       | 5/1988  | Erdman                                                                                                                                                                                                                                                                                                                                                                                                    |
| (65) | <b>Prior Publication Data</b>                                                                                                                                                                                                                                                                                                                                                               | 4,857,214 A       | 8/1989  | Papay et al.                                                                                                                                                                                                                                                                                                                                                                                              |
|      | US 2024/0199969 A1 Jun. 20, 2024                                                                                                                                                                                                                                                                                                                                                            | 4,925,983 A       | 5/1990  | Steckel                                                                                                                                                                                                                                                                                                                                                                                                   |
| (51) | <b>Int. Cl.</b>                                                                                                                                                                                                                                                                                                                                                                             | 4,956,122 A       | 9/1990  | Watts et al.                                                                                                                                                                                                                                                                                                                                                                                              |
|      | <b>C10M 129/42</b> (2006.01)                                                                                                                                                                                                                                                                                                                                                                | 4,992,183 A       | 2/1991  | Beimesch et al.                                                                                                                                                                                                                                                                                                                                                                                           |
|      | <b>C10M 129/72</b> (2006.01)                                                                                                                                                                                                                                                                                                                                                                | 5,089,156 A       | 2/1992  | Chrisope et al.                                                                                                                                                                                                                                                                                                                                                                                           |
|      | <b>C10M 169/04</b> (2006.01)                                                                                                                                                                                                                                                                                                                                                                | 5,114,602 A       | 5/1992  | Petrille et al.                                                                                                                                                                                                                                                                                                                                                                                           |
|      | <b>C10N 10/06</b> (2006.01)                                                                                                                                                                                                                                                                                                                                                                 | 5,614,480 A       | 3/1997  | Salomon et al.                                                                                                                                                                                                                                                                                                                                                                                            |
|      | <b>C10N 20/02</b> (2006.01)                                                                                                                                                                                                                                                                                                                                                                 | 6,124,247 A       | 9/2000  | Cazin et al.                                                                                                                                                                                                                                                                                                                                                                                              |
|      | <b>C10N 30/00</b> (2006.01)                                                                                                                                                                                                                                                                                                                                                                 | 6,303,546 B1      | 10/2001 | Hata et al.                                                                                                                                                                                                                                                                                                                                                                                               |
|      | <b>C10N 30/12</b> (2006.01)                                                                                                                                                                                                                                                                                                                                                                 | 2002/0165102 A1   | 11/2002 | Hata et al.                                                                                                                                                                                                                                                                                                                                                                                               |
|      | <b>C10N 40/25</b> (2006.01)                                                                                                                                                                                                                                                                                                                                                                 | 2004/0242434 A1   | 12/2004 | Yagishita et al.                                                                                                                                                                                                                                                                                                                                                                                          |
| (52) | <b>U.S. Cl.</b>                                                                                                                                                                                                                                                                                                                                                                             | 2005/0101496 A1   | 5/2005  | Loper et al.                                                                                                                                                                                                                                                                                                                                                                                              |
|      | CPC ..... <b>C10M 129/42</b> (2013.01); <b>C10M 129/72</b> (2013.01); <b>C10M 169/04</b> (2013.01); <b>C10M 2207/127</b> (2013.01); <b>C10M 2207/282</b> (2013.01); <b>C10N 2010/06</b> (2013.01); <b>C10N 2020/02</b> (2013.01); <b>C10N 2030/12</b> (2013.01); <b>C10N 2030/24</b> (2020.05); <b>C10N 2030/45</b> (2020.05); <b>C10N 2030/54</b> (2020.05); <b>C10N 2040/25</b> (2013.01) | 2006/0058200 A1   | 3/2006  | Shaw                                                                                                                                                                                                                                                                                                                                                                                                      |
| (58) | <b>Field of Classification Search</b>                                                                                                                                                                                                                                                                                                                                                       | 2006/0116302 A1   | 6/2006  | Deckman et al.                                                                                                                                                                                                                                                                                                                                                                                            |
|      | CPC ..... <b>C10M 129/42</b> ; <b>C10M 129/72</b> ; <b>C10M 169/04</b> ; <b>C10M 2207/127</b> ; <b>C10M 2207/282</b> ; <b>C10N 2030/24</b> ; <b>C10N 2030/54</b> ; <b>C10N 2030/45</b> ; <b>C10N 2010/06</b> ; <b>C10N 2020/02</b> ; <b>C10N 2030/12</b> ; <b>C10N 2040/25</b>                                                                                                              | 2006/0217271 A1   | 9/2006  | Brown et al.                                                                                                                                                                                                                                                                                                                                                                                              |
|      | See application file for complete search history.                                                                                                                                                                                                                                                                                                                                           | 2007/0184992 A1   | 8/2007  | Takeuchi et al.                                                                                                                                                                                                                                                                                                                                                                                           |
| (56) | <b>References Cited</b>                                                                                                                                                                                                                                                                                                                                                                     | 2008/0128184 A1   | 6/2008  | Loper et al.                                                                                                                                                                                                                                                                                                                                                                                              |
|      | <b>U.S. PATENT DOCUMENTS</b>                                                                                                                                                                                                                                                                                                                                                                | 2009/0156446 A1 * | 6/2009  | McAtee ..... C10M 141/10                                                                                                                                                                                                                                                                                                                                                                                  |
|      |                                                                                                                                                                                                                                                                                                                                                                                             |                   |         | 508/306                                                                                                                                                                                                                                                                                                                                                                                                   |
|      |                                                                                                                                                                                                                                                                                                                                                                                             | 2010/0029520 A1 * | 2/2010  | Kamano ..... C10M 141/10                                                                                                                                                                                                                                                                                                                                                                                  |
|      |                                                                                                                                                                                                                                                                                                                                                                                             |                   |         | 508/281                                                                                                                                                                                                                                                                                                                                                                                                   |
|      |                                                                                                                                                                                                                                                                                                                                                                                             | 2014/0187453 A1   | 7/2014  | Umeshara et al.                                                                                                                                                                                                                                                                                                                                                                                           |
|      |                                                                                                                                                                                                                                                                                                                                                                                             | 2014/0187455 A1   | 7/2014  | Umeshara et al.                                                                                                                                                                                                                                                                                                                                                                                           |
|      |                                                                                                                                                                                                                                                                                                                                                                                             | 2020/0140775 A1   | 5/2020  | Smith et al.                                                                                                                                                                                                                                                                                                                                                                                              |
|      |                                                                                                                                                                                                                                                                                                                                                                                             | 2020/0208074 A1   | 7/2020  | Jones et al.                                                                                                                                                                                                                                                                                                                                                                                              |
|      |                                                                                                                                                                                                                                                                                                                                                                                             | 2022/0010234 A1   | 1/2022  | Delbridge et al.                                                                                                                                                                                                                                                                                                                                                                                          |
|      |                                                                                                                                                                                                                                                                                                                                                                                             | 2022/0145206 A1   | 5/2022  | McBride et al.                                                                                                                                                                                                                                                                                                                                                                                            |
|      |                                                                                                                                                                                                                                                                                                                                                                                             |                   |         | FOREIGN PATENT DOCUMENTS                                                                                                                                                                                                                                                                                                                                                                                  |
|      |                                                                                                                                                                                                                                                                                                                                                                                             |                   |         | EP 0088453 A1 5/1987                                                                                                                                                                                                                                                                                                                                                                                      |
|      |                                                                                                                                                                                                                                                                                                                                                                                             |                   |         | EP 3056556 A1 8/2016                                                                                                                                                                                                                                                                                                                                                                                      |
|      |                                                                                                                                                                                                                                                                                                                                                                                             |                   |         | GB 961009 A 6/1964                                                                                                                                                                                                                                                                                                                                                                                        |
|      |                                                                                                                                                                                                                                                                                                                                                                                             |                   |         | OTHER PUBLICATIONS                                                                                                                                                                                                                                                                                                                                                                                        |
|      |                                                                                                                                                                                                                                                                                                                                                                                             |                   |         | Extended European Search Report issued in Application No. 23187291.2 mailed on Jan. 3, 2024, 9 pages.                                                                                                                                                                                                                                                                                                     |
|      |                                                                                                                                                                                                                                                                                                                                                                                             |                   |         | Extended European Search Report for EP 23214518.5, dated Jul. 19, 2024.                                                                                                                                                                                                                                                                                                                                   |
|      |                                                                                                                                                                                                                                                                                                                                                                                             |                   |         | * cited by examiner                                                                                                                                                                                                                                                                                                                                                                                       |
|      |                                                                                                                                                                                                                                                                                                                                                                                             |                   |         | Primary Examiner — Vishal V Vasisth                                                                                                                                                                                                                                                                                                                                                                       |
|      |                                                                                                                                                                                                                                                                                                                                                                                             |                   |         | (74) Attorney, Agent, or Firm — Honigman LLP                                                                                                                                                                                                                                                                                                                                                              |
|      |                                                                                                                                                                                                                                                                                                                                                                                             |                   |         | <b>ABSTRACT</b>                                                                                                                                                                                                                                                                                                                                                                                           |
|      |                                                                                                                                                                                                                                                                                                                                                                                             |                   |         | This disclosure describes low ash lubricating composition achieving passing steel corrosion, passing high temperature deposit formation, and emulsion stability. The lubricating compositions include one or more select corrosion or rust inhibitor chemistries having an oil-soluble acyclic structure with acidic, hydroxy, or amine moieties but being free of imine, imide, and/or amidine moieties. |
|      |                                                                                                                                                                                                                                                                                                                                                                                             |                   |         | <b>8 Claims, No Drawings</b>                                                                                                                                                                                                                                                                                                                                                                              |

## 1

LOW ASH LUBRICATING COMPOSITIONS  
FOR CONTROLLING STEEL CORROSION

## TECHNICAL FIELD

This disclosure relates to low ash additive systems and lubricating compositions including the additive systems configured for improved steel corrosion and emulsion stability and, in particular, low ash lubricating compositions with selected corrosion inhibitor chemistry capable of maintaining a stable emulsion and reducing or eliminating rust in steel corrosion performance testing.

## BACKGROUND

Automotive manufacturers continue to the push for improved efficiency and fuel economy, and as such, demands on engines, lubricants, and their components continue to increase. Today's passenger car engines are often smaller, lighter and more efficient with technologies designed to improve fuel economy, performance, and power. These requirements also mean engine oil performance must evolve to meet the higher demands of such modern engines and their corresponding performance criteria tied to their unique use and applications. With such exacting demands for engine oils, lubricant manufacturers often tailor lubricants and their additives to meet certain performance requirements for each unique application.

Lubricant specifications often include compositional constraints in terms of the permitted levels of sulfated ash, and maintaining such constraints while still meeting the heightened demands of the newest lubricant standards tends to be challenging. For example, it is often desired to lower the ash levels in a lubricant, but in some instances, lower ash levels tends to degrade other performance characteristics of the lubricant. For example, lower ash levels and associated changes to the lubricant compositions in view of the lower ash content can impact steel corrosion, high temperature deposits, and/or emulsion stability of the lubricants. Steel corrosion can be evaluated using various engine oil moisture corrosion tests, such as GMW 16073 and the like, emulsion stability can be evaluated, for instance, using the E85 emulsion test of ASTM D7563 or the like, and high temperature deposits can be evaluated using ASTM D6335 or the TEOST-33C test.

In many circumstances, however, varying one component within a lubricant composition to improve performance characteristics tends to negatively impact one or more other performance characteristics. For instance, the major sources of ash in a lubricating oil composition are generally metal detergent additives and/or anti-wear additives. However, it has been discovered that reducing the amount of ash content tends to negatively impact other performance characteristics, and in particular, lubricants with extreme low ash levels tends to degrade steel corrosion and/or cause problems with high temperature deposits. While use of corrosion inhibitors can be included in the lubricants to aid in steel corrosion performance, adding conventional corrosion inhibitors can, in some instances, degrade the emulsion stability of the lubricant.

## SUMMARY

In one approach or embodiment, a low-ash lubricating oil composition suitable for use in lubricating the engine of a passenger car is described. In approaches, the low-ash lubricating oil composition includes one or more base oils of

## 2

lubricating viscosity; a total sulfated ash (SASH) of about 0.5 weight percent or less; about 0.03 to about 0.2 weight percent of one or more acyclic corrosion inhibitors having an acidic, hydroxy, or amine moiety thereof and substantially free of compounds including imine, imide, amidine structural units or hydroxy derivatives thereof, and wherein the lubricating oil composition exhibits a stable emulsion at 0° C. and/or 25° C. pursuant to the E85 emulsion test of ASTM D7563 and no steel corrosion pursuant to the humidity corrosion test of GMW 16073.

In other approaches or embodiments, the low-ash lubricating oil composition described in the previous paragraph may include one or more optional features or embodiments.

These optional features or embodiments may include one or more of the following: wherein the one or more acyclic corrosion inhibitors includes an oil-soluble acid, diacid, acid-ester, polyol, amide, or mixtures thereof; and/or wherein the one or more acyclic corrosion inhibitors include a C6 or greater hydrocarbyl chain; and/or further comprising up to about 100 ppm of boron; and/or wherein the lubricating oil composition is substantially free of a metallic detergent; and/or wherein the lubricating oil composition has about 10 ppm or less of calcium, magnesium, or combinations thereof; and/or wherein the lubricating oil composition is substantially free of a metal dialkyldithiophosphate; and/or wherein the lubricating oil composition has about 10 ppm or less of zinc; and/or wherein the acyclic corrosion inhibitor is selected from (a) pentaerythritol mono-oleate, (b) N,N-dialkanol fatty amine, (c) C10 to C20 fatty amide, (d) C10 to C20 dicarboxylic acid, C10 to C20 acid-ester, or combinations thereof, or (e) condensation products of dodecenyl succinic acid or anhydride, or (f) mixtures thereof.

In another embodiment or approach, a low-ash lubricating oil composition suitable for use in lubricating the engine of a passenger car is also described herein wherein the low-ash lubricating oil composition includes one or more base oils of lubricating viscosity; a total calculated sulfated ash (SASH) of about 0.5 weight percent or less; up to about 0.3 weight percent of an acyclic corrosion inhibitor including one or more oil-soluble acids, diacids, acid-esters, or combinations thereof having a C6 or greater hydrocarbyl chain and being substantially free of compounds having imine, imide, amidine structural units or hydroxy derivatives thereof, and wherein the lubricating oil composition exhibits a stable emulsion at 0° C. and/or 25° C. pursuant to the E85 emulsion test of ASTM D7563 and no steel corrosion pursuant to the humidity corrosion test of GMW 16073.

In other embodiments or approaches, the low-ash lubricating oil composition described in the previous paragraph may also include one or more optional features or embodiments. These optional features or embodiment may include one or more of the following: further comprising up to about 100 ppm of boron; and/or wherein the lubricating oil composition is substantially free of a metallic detergent; and/or wherein the lubricating oil composition has about 10 ppm or less of calcium, magnesium, or combinations thereof, and/or wherein the lubricating oil composition is substantially free of a metal dialkyldithiophosphate; and/or wherein the lubricating oil composition has about 10 ppm or less of zinc; and/or wherein the acyclic corrosion inhibitor is one or more compounds having the structure of Formula I:



(Formula I)

and wherein each of  $R_1$  and  $R_2$  is, independently, selected from  $-\text{OH}$  or  $-\text{OR}_4\text{OH}$  with at least one of  $R_1$  and  $R_2$  being  $-\text{OH}$ ;  $R_3$  is a linear or branched C6 to C20 hydrocarbyl group; and  $R_4$  is a linear or branched C1 to C4 hydrocarbyl group with the  $-\text{OH}$  thereof being a primary or secondary alcohol; and/or wherein the acyclic corrosion inhibitor is a blend of an oil-soluble diacid and an oil-soluble acid-ester each having the structure of Formula I; and/or wherein the lubricating oil composition includes about 0.02 to about 0.3 weight percent of the acyclic corrosion inhibitor; and/or wherein the lubricating oil composition further has about 30 mg or less of deposits when subjected to the high temperature deposit formation test of ASTM D6335; and/or wherein the lubricating oil composition further has about 15 mg or less of deposits when subjected to the high temperature deposit formation test of ASTM D6335.

In yet other approaches or embodiments, the disclosure herein includes methods of lubricating a combustion engine using the low-ash lubricating oil compositions of this Summary and/or the use of any embodiment of the low-ash lubricating oil compositions as described in this Summary for achieving one or more of the following: a stable emulsion at  $0^\circ\text{C}$ . and/or  $25^\circ\text{C}$ . pursuant to the E85 emulsion test of ASTM D7563; no steel corrosion pursuant to the humidity corrosion test of GMW 16073; and/or about 30 mg or less of deposits when subjected to the high temperature deposit formation test of ASTM D6335.

Other embodiments of the present disclosure will be apparent to those skilled in the art from consideration of the specification and practice of the invention disclosed herein. The following definitions of terms are provided in order to clarify the meanings of certain terms as used herein.

The terms "oil composition," "lubrication composition," "lubricating oil composition," "lubricating oil," "lubricant composition," "lubricating composition," "fully formulated lubricant composition," "lubricant," "crankcase oil," "crankcase lubricant," "engine oil," "engine lubricant," "motor oil," and "motor lubricant" are considered synonymous, fully interchangeable terminology referring to the finished lubrication product comprising a major amount of a base oil plus a minor amount of an additive composition.

As used herein, the terms "additive package," "additive concentrate," "additive composition," "engine oil additive package," "engine oil additive concentrate," "crankcase additive package," "crankcase additive concentrate," "motor oil additive package," "motor oil concentrate," are considered synonymous, fully interchangeable terminology referring to the portion of the lubricating oil composition excluding the major amount of base oil stock mixture. The additive package may or may not include the viscosity index improver or pour point depressant.

The term "overbased" relates to metal salts, such as metal salts of sulfonates, carboxylates, salicylates, and/or phenates, wherein the amount of metal present exceeds the stoichiometric amount. Such salts may have a conversion level in excess of 100% (i.e., they may comprise more than

100% of the theoretical amount of metal needed to convert the acid to its "normal," "neutral" salt). The expression "metal ratio," often abbreviated as MR, is used to designate the ratio of total chemical equivalents of metal in the 5 overbased salt to chemical equivalents of the metal in a neutral salt according to known chemical reactivity and stoichiometry. In a normal or neutral salt, the metal ratio is one and in an overbased salt, MR, is greater than one. They are commonly referred to as overbased, hyperbased, or 10 superbased salts and may be salts of organic sulfur acids, carboxylic acids, salicylates, sulfonates, and/or phenols.

The term "alkaline earth metal" relates to calcium, barium, magnesium, and strontium, and the term "alkali metal" refers to lithium, sodium, potassium, rubidium, and 15 cesium.

As used herein, the term "hydrocarbyl" or "hydrocarbyl substituent" or "hydrocarbyl group" is used in its ordinary 20 sense, which is well-known to those skilled in the art. Specifically, it refers to a group having a carbon atom directly attached to the remainder of the molecule and having a predominantly hydrocarbon character. Each hydrocarbyl group is independently selected from hydrocarbon substituents, and substituted hydrocarbon substituents containing one or more of halo groups, hydroxyl groups, alkoxy groups, mercapto groups, nitro groups, nitroso groups, amino groups, pyridyl groups, furyl groups, imidazolyl groups, oxygen and nitrogen, and wherein no more than two non-hydrocarbon substituents are present for every ten carbon atoms in the hydrocarbyl group.

As used herein, the term "hydrocarbylene substituent" or "hydrocarbylene group" is used in its ordinary sense, which is well-known to those skilled in the art. Specifically, it refers to a group that is directly attached at two locations of 35 the molecule to the remainder of the molecule by a carbon atom and having predominantly hydrocarbon character. Each hydrocarbylene group is independently selected from divalent hydrocarbon substituents, and substituted divalent hydrocarbon substituents containing halo groups, alkyl groups, aryl groups, alkylaryl groups, arylalkyl groups, hydroxyl groups, alkoxy groups, mercapto groups, nitro groups, nitroso groups, amino groups, pyridyl groups, furyl groups, imidazolyl groups, oxygen and nitrogen, and wherein no more than two non-hydrocarbon substituents is 40 present for every ten carbon atoms in the hydrocarbylene group.

As used herein, the term "percent by weight", unless 45 expressly stated otherwise, means the percentage the recited component represents to the weight of the entire composition.

As used herein, the term "ppm" or "ppmw," unless expressly stated otherwise, refers to parts per million based on weight.

The terms "soluble," "oil-soluble," or "dispersible" used 55 herein may, but does not necessarily, indicate that the compounds or additives are soluble, dissolvable, miscible, or capable of being suspended in the oil in all proportions. The foregoing terms do mean, however, that they are, for instance, soluble, suspendable, dissolvable, or stably dispersible in oil to an extent sufficient to exert their intended effect in the environment in which the oil is employed. Moreover, the additional incorporation of other additives 60 may also permit incorporation of higher levels of a particular additive, if desired.

The term "TBN" as employed herein is used to denote the 65 Total Base Number in mg KOH/g as measured by the method of ASTM D2896.

The term "alkyl" as employed herein refers to straight, branched, cyclic, and/or substituted saturated chain moieties of from about 1 to about 100 carbon atoms. The term "alkenyl" as employed herein refers to straight, branched, cyclic, and/or substituted unsaturated chain moieties of from about 3 to about 10 carbon atoms. The term "aryl" as employed herein refers to single and multi-ring aromatic compounds that may include alkyl, alkenyl, alkylaryl, amino, hydroxyl, alkoxy, halo substituents, and/or heteroatoms including, but not limited to, nitrogen, oxygen, and sulfur.

As used herein, "post-reacted" or "post-treated" refers to a component that is further reacted with or treated with, for example, a boron, phosphorus, and/or maleic anhydride and may refer to dispersants in which primary and/or secondary amines are further reacted with such compounds to convert at least a portion of such amines to tertiary amines. Such subsequent reactions or treatments are further described in U.S. Pat. No. 5,241,003, which is incorporated herein by reference. Conversely, components that are "not post-reacted" or "not post-treated" have not been subjected to such further processing, reactions, and/or treatments and, in the context of dispersants, include a certain amount of primary and/or secondary amines.

The molecular weight for any embodiment herein may be determined with a gel permeation chromatography (GPC) instrument obtained from Waters or the like instrument and the data processed with Waters Empower Software or the like software. The GPC instrument may be equipped with a Waters Separations Module and Waters Refractive Index detector (or the like optional equipment). The GPC operating conditions may include a guard column, 4 Agilent PLgel columns (length of 300×7.5 mm; particle size of 5 $\mu$ , and pore size ranging from 100-10000 Å) with the column temperature at about 40° C. Un-stabilized HPLC grade tetrahydrofuran (THF) may be used as solvent, at a flow rate of 1.0 mL/min. The GPC instrument may be calibrated with commercially available polystyrene (PS) standards having a narrow molecular weight distribution ranging from 500-380,000 g/mol. The calibration curve can be extrapolated for samples having a mass less than 500 g/mol. Samples and PS standards can be in dissolved in THF and prepared at concentration of 0.1 to 0.5 wt. % and used without filtration. GPC measurements are also described in U.S. Pat. No. 5,266,223, which is incorporated herein by reference. The GPC method additionally provides molecular weight distribution information; see, for example, W. W. Yau, J. J. Kirkland and D. D. Bly, "Modern Size Exclusion Liquid Chromatography", John Wiley and Sons, New York, 1979, also incorporated herein by reference.

As used herein, "sulfated ash" or "SASH" refers to the amount of sulfated ash as measured using ASTM D874. Alternatively, sulfated ash may also be calculated based on the amount of metals in the lubricant. For example, sulfated ash (SASH) may optionally be calculated based on the total metallic elements that contribute to SASH in the lubricant composition adjusted by factors for each metallic type. The metals that contribute to SASH include (along with the adjustment factor) barium (1.7), boron (3.22), calcium (3.4), copper (1.252), lead (1.464), lithium (7.92), magnesium (4.95), manganese (1.291), molybdenum (1.5), potassium (2.33), sodium (3.09), and zinc (1.5). Specifically, the ppmw content of each of the metallic elements present in a lubricating oil composition that is considered to contribute to sulfated ash is multiplied by its corresponding factor above; then, the product for each metallic element/factor adjustment is summed and the total is divided by 10,000 to

calculate the weight percent of SASH in the lubricating compositions. Unless specified otherwise, all sulfated ash levels herein are measured using ASTM D874.

Additional details and advantages of the disclosure will be set forth in part in the description that follows, and/or may be learned by practice of the disclosure. The details and advantages of the disclosure may be realized and attained by means of the elements and combinations particularly pointed out in the appended claims. It is to be understood that both the foregoing general description and the following detailed description are exemplary and explanatory only and are not restrictive of the disclosure, as claimed.

#### DETAILED DESCRIPTION

15 Sulfated ash is a measurement that indicates the total weight percent of ash in a lubricating oil composition. The sulfated ash measurement for a lubricating oil composition is related to the total metal content therein and may be 20 conveniently measured according to ASTM D874 and/or other common evaluation methods known in the art and as described herein. In one aspect, this disclosure describes additives and lubricants including such additives providing extremely low sulfated ash (SASH) content of about 0.5 25 weight percent or less, about 0.3 weight percent or less, or 0.1 weight percent or less. As shown in the Examples below, when a lubricant is modified to have such extreme low sulfated ash levels, it becomes difficult to achieve passing steel corrosion performance (GMW 16073) and/or passing 30 high temperature deposit formation (ASTM D6335).

35 While the conventional approach would be to include a rust or corrosion inhibitor to improve the steel corrosion performance, use of conventional corrosion inhibitors do not necessarily improve steel corrosion performance in the 40 context of such extreme low levels of ash, and even if steel corrosion performance is improved, it was unexpected that certain conventional corrosion inhibitors would then cause the lubricants to fail E85 emulsion stability. For instance, 45 select chemistries of oil-soluble imine, imide, or amidine compounds (or hydroxy derivatives thereof) may improve steel corrosion performance and achieve passing high temperature deposits, but such chemistries then degrade the lubricant's emulsion stability. Surprisingly, careful selection 50 of the chemistry forming the oil-soluble corrosion or rust inhibitors can improve both steel corrosion and, at the same time, maintain emulsion stability and low levels of high temperature deposits. For instance, select corrosion or rust inhibitor chemistries having an oil-soluble acyclic structure with acidic, hydroxy, or amine moieties surprisingly improves steel corrosion, maintains emulsion stability, and achieves low levels of high temperature deposits.

In one embodiment, about 0.03 to about 0.2 weight 55 percent of oil-soluble acyclic compounds having one or more acidic, hydroxy, and/or amine moieties provide desired steel corrosion, passing high temperature deposits, and emulsion stability in extreme low ash lubricants, but only when the oil-soluble compounds were also substantially free of imine, imide, and/or amidine structural units. In another embodiment or approach herein, up to about 0.3 weight 60 percent (preferably, about 0.02 to about 0.3 weight percent) of an acyclic compound including one or more oil-soluble acids, diacids, acid-esters, or combinations thereof having a C6 or greater hydrocarbyl group providing the oil solubility achieved the desired level of steel corrosion, passing high temperature deposits, and emulsion stability, but again only when such oil-soluble compounds were also substantially free of imine, imide, and/or amidine structural units.

Turning to more of the specifics, the oil-soluble rust or corrosion inhibitor compounds herein may include acyclic compounds having the acidic, hydroxy, or amine moieties, but also being substantially free of imine, imide, or amidine structural units. In one approach, for instance, the extreme low-ash lubricating oil compositions herein include one or more acyclic compounds including an oil-soluble acid, diacid, acid-ester, polyol, amide and/or mixtures thereof. The one or more acyclic compounds may include at least one C6 or greater hydrocarbyl chain, a C8 or greater hydrocarbyl chain, or a C10 or greater hydrocarbyl chain to provide the oil-solubility. The upper end of the hydrocarbyl chain for oil-solubility is not particularly limited, but may be a C50 or less hydrocarbyl chain, a C40 or less hydrocarbyl chain, a C30 or less hydrocarbyl chain, a C25 or less hydrocarbyl chain, or a C20 or less hydrocarbyl chain.

In some approaches or embodiments, the oil-soluble acyclic compound may be one or more aliphatic polyhydric alcohols having 2 to 10 hydroxy groups, in another approach 2 to 8 hydroxy groups, or in yet a further approach 2 to 4 hydroxy group. In one particular approach or embodiment, the oil-soluble acyclic compound is pentaerythritol monooleate. The lubricants herein may include about 0.03 to about 0.3 weight percent of such polyhydric alcohols, and preferably, about 0.05 to about 0.3 weight percent.

In another approach or embodiment, the oil-soluble acyclic compound may also be one or more fatty amines such as oil-soluble saturated or unsaturated alkylated amines and may be a monoamine (with a terminal primary amine) or a polyamine. Suitable fatty amines include N,N-dialkanol fatty amines or, more preferably, N,N-diethanol tallow amine. The lubricants herein may include about 0.02 to about 0.2 weight percent of such fatty amines, and more preferably, about 0.02 to about 0.175 weight percent of the fatty amines.

In yet another approach or embodiment, the oil-soluble acyclic compound may also include one or more fatty amide compounds such as saturated or unsaturated fatty amides including C10 to C20 unsaturated fatty amides and, preferably, is an amide of oleic acid. The lubricants herein may include about 0.02 to about 0.3 weight percent of such fatty amides.

In further approaches or embodiments, the oil-soluble acyclic compounds may also include oil-soluble diacids, oil-soluble acid-esters or half esters, or combinations thereof. In a particular approach or embodiment, the oil-soluble acyclic compound may include C10 to C20 dicarboxylic acids, C10 to C20 acid-esters, or combinations thereof. The lubricants herein may include about 0.02 to about 0.3 weight percent of such diacid and acid-ester compounds or blends thereof.

In one particular approach or embodiment, the oil-soluble acyclic compound is one or more diacid and/or acid-ester compounds having the structure of Formula I:



(Formula I)

wherein each of R<sub>1</sub> and R<sub>2</sub> is, independently, selected from —OH or —OR<sub>4</sub>OH with at least one of R<sub>1</sub> and R<sub>2</sub> being —OH; R<sub>3</sub> is a linear or branched oil-soluble hydrocarbyl group, preferably a C6 to C50 hydrocarbyl group (more preferably, a C6 to C20 hydrocarbyl group); and R<sub>4</sub> is a linear or branched C1 to C4 hydrocarbyl group wherein the associated —OH group is one of a primary or secondary alcohol. In some approaches, the oil-soluble acyclic corrosion inhibitor is a blend of an oil-soluble diacid and an oil-soluble acid-ester each having the structure of Formula I. In some approaches, the lubricating oil compositions herein includes about 0.02 to about 0.3 weight percent of the acyclic compounds of Formula I in the extreme low ash formulations having a sulfated ash content of about 0.5 weight percent or below (about 0.3 weight percent or below or about 0.1 weight percent or below) as noted above.

In other approaches or embodiments, the oil-soluble acyclic compounds herein may also include condensation products of dodecenyl succinic acid or anhydride and may include about 0.03 to about 0.3 weight percent or, preferably about 0.05 to about 0.3 weight percent.

The oil-soluble acyclic compounds herein may also be a mixture of any combination of the above described rust or corrosion inhibitors.

Surprisingly, oil-soluble compounds having an imine, imide, or amidine structural units (or hydroxy derivatives thereof) that are commonly used as rust or corrosion inhibitors fail either the steel corrosion tests and/or the emulsion stability tests when included in extreme low ash lubricants. The oil-soluble corrosion inhibitors herein are also free of rust or corrosion inhibitors having aromatic moieties or other aryl derivatives thereof. Thus, the lubricants herein are substantially free of oil-soluble compounds including imine, imide, amidine, or aromatic structural units or hydroxyl derivatives thereof. As used herein, substantially free of means less than about 0.1 weight percent, less than about 0.05 weight percent, less than about 0.02 weight percent, less than about 0.01 weight percent, less than about 0.005 weight percent, or no oil-soluble compounds including one or more of an imine, imide, aromatic, and/or amidine moieties and/or any hydroxy derivatives thereof.

#### The Extreme Low-Ash System

As noted above, the lubricant compositions herein are formulated to have extremely low levels of sulfated ash, and include an additive package providing a composition with sulfated ash levels (ASTM D874) of about 0.5 weight percent or less, about 0.3 weight percent or less, about 0.2 weight percent or less, about 0.1 weight percent or less, about 0.08 weight percent or less, about 0.07 weight percent or less, or about 0.06 weight percent or less (ASTM D874). In other approaches, the lubricant compositions herein may also include about 0.01 weight percent or more of sulfated ash, about 0.02 weight percent or more, about 0.3 weight percent or more, or about 0.04 weight percent or more of sulfated ash (ASTM D874).

To achieve such extremely low content of sulfated ash, the lubricant compositions herein have a select additive package providing an additive mixture with only select amounts of compounds providing boron, calcium, magnesium, molybdenum, and/or zinc. To this end, the lubricants herein preferably include additives providing one or more of the following: no more than about 100 ppm of boron, no more than about 100 ppm of calcium, no more than about 100 ppm of magnesium, no more than about 100 ppm of molybdenum, and no more than about 100 ppm of zinc, and/or any combination thereof. Preferably, the lubricating oil compositions herein include additives providing about 10 ppm or

less of each of calcium, magnesium, zinc, molybdenum, and/or combinations thereof together with additives providing no more than about 100 ppm of boron (preferably no more than about 80 ppm of boron, no more than about 60 ppm of boron). In other approaches, the lubricating compositions herein are substantially free of metallic detergents and, more preferably, the lubricating composition have metal detergents providing less than about 100 ppm of total detergent metals, less than 80 ppm of total detergent metals, less than 50 ppm of total detergent metals, less than 20 ppm of total detergent metals, or less than 10 ppm of total detergent metals where detergent metals are selected from calcium, magnesium, and the like. In other approaches, the lubricating oil compositions herein are also substantially free of metal dialkyldithiophosphates (such as zinc dialkyldithiophosphates) and, in such context, preferably have about 10 ppm or less of zinc provided by such metal dialkyldithiophosphate.

#### Lubricating Oil Compositions

The one or more acyclic rust or corrosion inhibitors described above may be combined with a major amount of a base oil or base oil blend of lubricating viscosity (as described below) in combination with one or more further optional additives to produce a lubricating oil composition. In approaches, the lubricating oil compositions includes about 50 weight percent or more of the base oil blend, about 60 weight percent or more, about 70 weight percent or more, or about 80 weight percent or more to about 95 weight percent or less, about 90 weight percent or less, about 85 weight percent or less of the base oil blend as such blend is further discussed below. The lubricating compositions herein may have a KV100 of about 2 to about 15 cSt (ASTM D445), and preferably, about 5 to about 12 cSt, and more preferably 5 to about 10 cSt.

When the lubricating compositions herein include such extreme low levels of sulfated ash combined with the select acyclic rust or corrosion inhibitors, the lubricating compositions herein have less than about 30 mg of deposits when subjected to the high temperature deposit formation test of ASTM D6335 (TEOST-33C), achieve no corrosion pursuant to an engine oil moisture corrosion test such as GMW 16073, and maintain a stable emulsion with no water separation pursuant to ASTM D7563 at both 0° C. and 25° C.

**Base Oil Blend:** The base oil used in the lubricating oil compositions herein may be oils of lubricating viscosity and selected from any of the base oils in Groups I-V as specified in the American Petroleum Institute (API) Base Oil Interchangeability Guidelines. The five base oil groups are as follows:

TABLE 1

| Base oil Category | Sulfur (%)                                          | Saturates (%) | Viscosity Index |
|-------------------|-----------------------------------------------------|---------------|-----------------|
| Group I           | >0.03                                               | and/or        | <90             |
| Group II          | ≤0.03                                               | and           | ≥90             |
| Group III         | ≤0.03                                               | and           | ≥90             |
| Group IV          | All polyalphaolefins (PAOs)                         |               |                 |
| Group V           | All others not included in Groups I, II, III, or IV |               |                 |

Groups I, II, and III are mineral oil process stocks. Group IV base oils contain true synthetic molecular species, which are produced by polymerization of olefinically unsaturated hydrocarbons. Many Group V base oils are also true synthetic products and may include diesters, polyol esters, polyalkylene glycols, alkylated aromatics, polyphosphate esters, polyvinyl ethers, and/or polyphenyl ethers, and the

like, but may also be naturally occurring oils, such as vegetable oils. It should be noted that although Group III base oils are derived from mineral oil, the rigorous processing that these fluids undergo causes their physical properties to be very similar to some true synthetics, such as PAOs. Therefore, oils derived from Group III base oils may be referred to as synthetic fluids in the industry. Group II+ may comprise high viscosity index Group II.

The base oil blend used in the disclosed lubricating oil composition may be a mineral oil, animal oil, vegetable oil, synthetic oil, synthetic oil blends, or mixtures thereof. Suitable oils may be derived from hydrocracking, hydrogeneration, hydrofinishing, unrefined, refined, and re-refined oils, and mixtures thereof.

Unrefined oils are those derived from a natural, mineral, or synthetic source without or with little further purification treatment. Refined oils are similar to the unrefined oils except that they have been treated in one or more purification steps, which may result in the improvement of one or more properties. Examples of suitable purification techniques are solvent extraction, secondary distillation, acid or base extraction, filtration, percolation, and the like. Oils refined to the quality of an edible may or may not be useful. Edible oils may also be called white oils. In some embodiments, lubricating oil compositions are free of edible or white oils.

Re-refined oils are also known as reclaimed or reprocessed oils. These oils are obtained similarly to refined oils using the same or similar processes. Often these oils are additionally processed by techniques directed to removal of spent additives and oil breakdown products.

Mineral oils may include oils obtained by drilling or from plants and animals or any mixtures thereof. For example such oils may include, but are not limited to, castor oil, lard oil, olive oil, peanut oil, corn oil, soybean oil, and linseed oil, as well as mineral lubricating oils, such as liquid petroleum oils and solvent-treated or acid-treated mineral lubricating oils of the paraffinic, naphthenic or mixed paraffinic-naphthenic types. Such oils may be partially or fully hydrogenated, if desired. Oils derived from coal or shale may also be useful.

Useful synthetic lubricating oils may include hydrocarbon oils such as polymerized, oligomerized, or interpolymerized olefins (e.g., polybutylenes, polypropylenes, propyleneisobutylene copolymers); poly(1-hexenes), poly(1-octenes), trimers or oligomers of 1-decene, e.g., poly(1-decenes), such materials being often referred to as  $\alpha$ -olefins, and mixtures thereof; alkyl-benzenes (e.g. dodecylbenzenes,

60 tetradecylbenzenes, dinonylbenzenes, di-(2-ethylhexyl)-benzenes); polyphenyls (e.g., biphenyls, terphenyls, alkylated polyphenyls); diphenyl alkanes, alkylated diphenyl alkanes, alkylated diphenyl ethers and alkylated diphenyl sulfides and the derivatives, analogs and homologs thereof or mixtures thereof. Polyalphaolefins are typically hydrogenated materials.

## 11

Other synthetic lubricating oils include polyol esters, diesters, liquid esters of phosphorus-containing acids (e.g., tricresyl phosphate, trioctyl phosphate, and the diethyl ester of decane phosphonic acid), or polymeric tetrahydrofurans. Synthetic oils may be produced by Fischer-Tropsch reactions and typically may be hydroisomerized Fischer-Tropsch hydrocarbons or waxes. In one embodiment oils may be prepared by a Fischer-Tropsch gas-to-liquid synthetic procedure as well as other gas-to-liquid oils.

The major amount of base oil included in a lubricating composition may be selected from the group consisting of Group I, Group II, a Group III, a Group IV, a Group V, and a combination of two or more of the foregoing, and wherein the major amount of base oil is other than base oils that arise from provision of additive components or viscosity index improvers in the composition. In another embodiment, the major amount of base oil included in a lubricating composition may be selected from the group consisting of Group II, a Group III, a Group IV, a Group V, and a combination of two or more of the foregoing, and wherein the major amount of base oil is other than base oils that arise from provision of additive components or viscosity index improvers in the composition.

The amount of the oil of lubricating viscosity present may be the balance remaining after subtracting from 100 wt % the sum of the amount of the performance additives inclusive of viscosity index improver(s) and/or pour point depressant(s) and/or other top treat additives. For example, the oil of lubricating viscosity that may be present in a finished fluid may be a major amount, such as greater than about 50 wt %, greater than about 60 wt %, greater than about 70 wt %, greater than about 80 wt %, greater than about 85 wt %, or greater than about 90 wt %.

## Optional Additives:

The lubricating oil compositions herein may also include a number of optional additives combined with the acyclic rust or corrosion inhibitors discussed above as needed to meet performance standards so long as the noted relationships for the sulfated ash and composition of the rust or corrosion inhibitors discussed above is maintained. Those optional additives are described in the following paragraphs.

**Dispersants:** The lubricating oil composition may optionally include one or more dispersants or mixtures thereof. Dispersants are often known as ashless-type dispersants because, prior to mixing in a lubricating oil composition, they do not contain ash-forming metals and they do not normally contribute any ash when added to a lubricant. Ashless type dispersants are characterized by a polar group attached to a relatively high molecular weight hydrocarbon chain. Typical ashless dispersants include N-substituted long chain alkenyl succinimides. Examples of N-substituted long chain alkenyl succinimides include polyisobutylene succinimide with the number average molecular weight of the polyisobutylene substituent being in the range about 350 to about 50,000, or to about 5,000, or to about 3,000, as measured by GPC. Succinimide dispersants and their preparation are disclosed, for instance in U.S. Pat. No. 7,897,696 or U.S. Pat. No. 4,234,435. The alkenyl substituent may be prepared from polymerizable monomers containing about 2 to about 16, or about 2 to about 8, or about 2 to about 6 carbon atoms. Succinimide dispersants are typically the imide formed from a polyamine, typically a poly(ethylene amine).

Preferred amines are selected from polyamines and hydroxyamines. Examples of polyamines that may be used include, but are not limited to, diethylene triamine (DETA), triethylene tetramine (TETA), tetraethylene pentamine

## 12

(TEPA), and higher homologues such as pentaethylene hexamine (PEHA), and the like.

A suitable heavy polyamine is a mixture of polyalkylene-polyamines comprising small amounts of lower polyamine oligomers such as TEPA and PEHA (pentaethylene hexamine) but primarily oligomers with 6 or more nitrogen atoms, 2 or more primary amines per molecule, and more extensive branching than conventional polyamine mixtures. A heavy polyamine preferably includes polyamine oligomers containing 7 or more nitrogen atoms per molecule and with 2 or more primary amines per molecule. The heavy polyamine comprises more than 28 wt. % (e.g. >32 wt. %) total nitrogen and an equivalent weight of primary amine groups of 120-160 grams per equivalent.

In some approaches, suitable polyamines are commonly known as PAM and contain a mixture of ethylene amines where TEPA and pentaethylene hexamine (PEHA) are the major part of the polyamine, usually less than about 80%.

Typically, PAM has 8.7-8.9 milliequivalents of primary amine per gram (an equivalent weight of 115 to 112 grams per equivalent of primary amine) and a total nitrogen content of about 33-34 wt. %. Heavier cuts of PAM oligomers with practically no TEPA and only very small amounts of PEHA but containing primarily oligomers with more than 6 nitrogen atoms and more extensive branching, may produce dispersants with improved dispersancy.

In an embodiment the present disclosure further comprises at least one polyisobutylene succinimide dispersant derived from polyisobutylene with a number average molecular weight in the range about 350 to about 50,000, or to about 5000, or to about 3000, as determined by GPC. The polyisobutylene succinimide may be used alone or in combination with other dispersants.

In some embodiments, polyisobutylene, when included, may have greater than 50 mol %, greater than 60 mol %, greater than 70 mol %, greater than 80 mol %, or greater than 90 mol % content of terminal double bonds. Such PIB is also referred to as highly reactive PIB ("HR-PIB"). HR-PIB having a number average molecular weight ranging from about 800 to about 5000, as determined by GPC, is suitable for use in embodiments of the present disclosure. Conventional PIB typically has less than 50 mol %, less than 40 mol %, less than 30 mol %, less than 20 mol %, or less than 10 mol % content of terminal double bonds.

An HR-PIB having a number average molecular weight ranging from about 900 to about 3000 may be suitable, as determined by GPC. Such HR-PIB is commercially available, or can be synthesized by the polymerization of isobutene in the presence of a non-chlorinated catalyst such as boron trifluoride, as described in U.S. Pat. No. 4,152,499 to Boerzel, et al. and U.S. Pat. No. 5,739,355 to Gateau, et al. When used in the aforementioned thermal ene reaction, HR-PIB may lead to higher conversion rates in the reaction, as well as lower amounts of sediment formation, due to increased reactivity. A suitable method is described in U.S. Pat. No. 7,897,696.

In one embodiment, the present disclosure further comprises at least one dispersant derived from polyisobutylene succinic anhydride ("PIBSA"). The PIBSA may have an average of between about 1.0 and about 2.0 succinic acid moieties per polymer.

The % actives of the alkenyl or alkyl succinic anhydride can be determined using a chromatographic technique. This method is described in column 5 and 6 in U.S. Pat. No. 5,334,321.

## 13

The percent conversion of the polyolefin is calculated from the % actives using the equation in column 5 and 6 in U.S. Pat. No. 5,334,321.

Unless stated otherwise, all percentages are in weight percent and all molecular weights are number average molecular weights determined by gel permeation chromatography (GPC) using commercially available polystyrene standards (with a number average molecular weight of 180 to about 18,000 as the calibration reference).

In one embodiment, the dispersant may be derived from a polyalphaolefin (PAO) succinic anhydride. In one embodiment, the dispersant may be derived from olefin maleic anhydride copolymer. As an example, the dispersant may be described as a poly-PIBSA. In an embodiment, the dispersant may be derived from an anhydride which is grafted to an ethylene-propylene copolymer.

A suitable class of nitrogen-containing dispersants may be derived from olefin copolymers (OCP), more specifically, ethylene-propylene dispersants which may be grafted with maleic anhydride. A more complete list of nitrogen-containing compounds that can be reacted with the functionalized OCP are described in U.S. Pat. Nos. 7,485,603; 7,786,057; 7,253,231; 6,107,257; and 5,075,383; and/or are commercially available.

One class of suitable dispersants may also be Mannich bases. Mannich bases are materials that are formed by the condensation of a higher molecular weight, alkyl substituted phenol, a polyalkylene polyamine, and an aldehyde such as formaldehyde. Mannich bases are described in more detail in U.S. Pat. No. 3,634,515.

A suitable class of dispersants may also be high molecular weight esters or half ester amides. A suitable dispersant may also be post-treated by conventional methods by a reaction with any of a variety of agents. Among these are boron, urea, thiourea, dimercaptodiimidazoles, carbon disulfide, aldehydes, ketones, carboxylic acids, hydrocarbon-substituted succinic anhydrides, maleic anhydride, nitriles, epoxides, carbonates, cyclic carbonates, hindered phenolic esters, and phosphorus compounds. U.S. Pat. Nos. 7,645,726; 7,214,649; and 8,048,831 are incorporated herein by reference in their entireties.

In addition to the carbonate and boric acids post-treatments both the compounds may be post-treated, or further post-treatment, with a variety of post-treatments designed to improve or impart different properties. Such post-treatments include those summarized in columns 27-29 of U.S. Pat. No. 5,241,003, hereby incorporated by reference. Such treatments include, treatment with: Inorganic phosphorous acids or anhydrides (e.g., U.S. Pat. Nos. 3,403,102 and 4,648,980); Organic phosphorous compounds (e.g., U.S. Pat. No. 3,502,677); Phosphorous pentasulfides; Boron compounds as already noted above (e.g., U.S. Pat. Nos. 3,178,663 and 4,652,387); Carboxylic acid, polycarboxylic acids, anhydrides and/or acid halides (e.g., U.S. Pat. Nos. 3,708,522 and 4,948,386); Epoxides polyepoxides or thioepoxides (e.g., U.S. Pat. Nos. 3,859,318 and 5,026,495); Aldehyde or ketone (e.g., U.S. Pat. No. 3,458,530); Carbon disulfide (e.g., U.S. Pat. No. 3,256,185); Glycidol (e.g., U.S. Pat. No. 4,617,137); Urea, thiourea or guanidine (e.g., U.S. Pat. Nos. 3,312,619; 3,865,813; and British Patent GB 1,065,595); Organic sulfonic acid (e.g., U.S. Pat. No. 3,189,544 and British Patent GB 2,140,811); Alkenyl cyanide (e.g., U.S. Pat. Nos. 3,278,550 and 3,366,569); Diketene (e.g., U.S. Pat. No. 3,546,243); A diisocyanate (e.g., U.S. Pat. No. 3,573,205); Alkane sulfone (e.g., U.S. Pat. No. 3,749,695); 1,3-Dicarbonyl Compound (e.g., U.S. Pat. No. 4,579,675); Sulfate of alkoxylated alcohol or phenol (e.g., U.S. Pat. No.

## 14

3,954,639); Cyclic lactone (e.g., U.S. Pat. Nos. 4,617,138; 4,645,515; 4,668,246; 4,963,275; and 4,971,711); Cyclic carbonate or thiocarbonate linear monocarbonate or polycarbonate, or chloroformate (e.g., U.S. Pat. Nos. 4,612,132; 4,647,390; 4,648,886; 4,670,170); Nitrogen-containing carboxylic acid (e.g., U.S. Pat. No. 4,971,598 and British Patent GB 2,140,811); Hydroxy-protected chlorodicarbonyloxy compound (e.g., U.S. Pat. No. 4,614,522); Lactam, thiolactam, thiolactone or dithiolactone (e.g., U.S. Pat. Nos. 4,614,603 and 4,666,460); Cyclic carbamate, cyclic thiocarbamate or cyclic dithiocarbamate (e.g., U.S. Pat. Nos. 4,663,062 and 4,666,459); Hydroxyaliphatic carboxylic acid (e.g., U.S. Pat. Nos. 4,482,464; 4,521,318; 4,713,189); Oxidizing agent (e.g., U.S. Pat. No. 4,379,064); Combination of phosphorus pentasulfide and a polyalkylene polyamine (e.g., U.S. Pat. No. 3,185,647); Combination of carboxylic acid or an aldehyde or ketone and sulfur or sulfur chloride (e.g., U.S. Pat. Nos. 3,390,086; 3,470,098); Combination of a hydrazine and carbon disulfide (e.g., U.S. Pat. No. 3,519,564); Combination of an aldehyde and a phenol (e.g., U.S. Pat. Nos. 3,649,229; 5,030,249; 5,039,307); Combination of an aldehyde and an O-diester of dithiophosphoric acid (e.g., U.S. Pat. No. 3,865,740); Combination of a hydroxyaliphatic carboxylic acid and a boric acid (e.g., U.S. Pat. No. 4,554,086); Combination of a hydroxyaliphatic carboxylic acid, then formaldehyde and a phenol (e.g., U.S. Pat. No. 4,636,322); Combination of a hydroxyaliphatic carboxylic acid and then an aliphatic dicarboxylic acid (e.g., U.S. Pat. No. 4,663,064); Combination of formaldehyde and a phenol and then glycolic acid (e.g., U.S. Pat. No. 4,699,724); Combination of a hydroxyaliphatic carboxylic acid or oxalic acid and then a diisocyanate (e.g., U.S. Pat. No. 4,713,191); Combination of inorganic acid or anhydride of phosphorus or a partial or total sulfur analog thereof and a boron compound (e.g., U.S. Pat. No. 4,857,214); Combination of an organic diacid then an unsaturated fatty acid and then a nitroaromatic amine optionally followed by a boron compound and then a glycolating agent (e.g., U.S. Pat. No. 4,973,412); Combination of an aldehyde and a triazole (e.g., U.S. Pat. No. 4,963,278); Combination of an aldehyde and a triazole then a boron compound (e.g., U.S. Pat. No. 4,981,492); Combination of cyclic lactone and a boron compound (e.g., U.S. Pat. Nos. 4,963,275 and 4,971,711). The above-mentioned patents are herein incorporated in their entireties.

55 The TBN of a suitable dispersant may be from about 10 to about 65 mg KOH/g dispersant, on an oil-free basis, which is comparable to about 5 to about 30 TBN if measured on a dispersant sample containing about 50% diluent oil. TBN is measured by the method of ASTM D2896.

60 In yet other embodiments, the optional dispersant additive may be a hydrocarbyl substituted succinamide or succinimide dispersant. In approaches, the hydrocarbyl substituted succinamide or succinimide dispersant may be derived from a hydrocarbyl substituted acylating agent reacted with a polyalkylene polyamine and wherein the hydrocarbyl substituent of the succinamide or the succinimide dispersant is a linear or branched hydrocarbyl group having a number

average molecular weight of about 250 to about 5,000 as measured by GPC using polystyrene as a calibration reference.

In some approaches, the polyalkylene polyamine used to form the dispersant has the



wherein each R and R', independently, is a divalent C1 to C6 alkylene linker, each R<sub>1</sub> and R<sub>2</sub>, independently, is hydrogen, a C1 to C6 alkyl group, or together with the nitrogen atom to which they are attached form a 5- or 6-membered ring optionally fused with one or more aromatic or non-aromatic rings, and n is an integer from 0 to 8. In other approaches, the polyalkylene polyamine is selected from the group consisting of a mixture of polyethylene polyamines having an average of 5 to 7 nitrogen atoms, triethylenetetramine, tetraethylenepentamine, and combinations thereof.

The dispersant, if present, can be used in an amount sufficient to provide up to about 20 wt %, based upon the final weight of the lubricating oil composition. Another amount of the dispersant that can be used may be about 0.1 wt % to about 15 wt %, or about 0.1 wt % to about 10 wt %, about 0.1 to 8 wt %, or about 1 wt % to about 10 wt %, or about 1 wt % to about 8 wt %, or about 1 wt % to about 6 wt %, based upon the final weight of the lubricating oil composition. In some embodiments, the lubricating oil composition utilizes a mixed dispersant system. A single type or a mixture of two or more types of dispersants in any desired ratio may be used.

**Antioxidants:** The lubricating oil compositions herein also may optionally contain antioxidants. Antioxidant compounds are known and include for example, phenates, phenate sulfides, sulfurized olefins, phosphosulfurized terpenes, sulfurized esters, aromatic amines, alkylated diphenylamines (e.g., nonyl diphenylamine, di-nonyl diphenylamine, octyl diphenylamine, di-octyl diphenylamine), phenyl-alpha-naphthylamines, alkylated phenyl-alpha-naphthylamines, hindered non-aromatic amines, phenols, hindered phenols, oil-soluble molybdenum compounds, macromolecular antioxidants, or mixtures thereof. Antioxidant compounds may be used alone or in combination.

The hindered phenol antioxidant may contain a secondary butyl and/or a tertiary butyl group as a sterically hindering group. The phenol group may be further substituted with a hydrocarbyl group and/or a bridging group linking to a second aromatic group. Examples of suitable hindered phenol antioxidants include 2,6-di-tert-butylphenol, 4-methyl-2,6-di-tert-butylphenol, 4-ethyl-2,6-di-tert-butylphenol, 4-propyl-2,6-di-tert-butylphenol or 4-butyl-2,6-di-tert-butylphenol, or 4-dodecyl-2,6-di-tert-butylphenol. In one embodiment the hindered phenol antioxidant may be an ester and may include, e.g., Irganox<sup>TM</sup> L-135 available from BASF or an addition product derived from 2,6-di-tert-butylphenol and an alkyl acrylate, wherein the alkyl group may contain about 1 to about 18, or about 2 to about 12, or about 2 to about 8, or about 2 to about 6, or about 4 carbon atoms. Another commercially available hindered phenol antioxidant may be an ester and may include Ethanol<sup>TM</sup> 4716 available from Albemarle Corporation.

Useful antioxidants may include diarylamines and high molecular weight phenols. In an embodiment, the lubricat-

ing oil composition may contain a mixture of a diarylamine and a high molecular weight phenol, such that each antioxidant may be present in an amount sufficient to provide up to about 5%, by weight, based upon the final weight of the lubricating oil composition. In an embodiment, the antioxidant may be a mixture of about 0.3 to about 1.5% diarylamine and about 0.4 to about 2.5% high molecular weight phenol, by weight, based upon the final weight of the lubricating oil composition.

Examples of suitable olefins that may be sulfurized to form a sulfurized olefin include propylene, butylene, isobutylene, polyisobutylene, pentene, hexene, heptene, octene, nonene, decene, undecene, dodecene, tridecene, tetradecene, pentadecene, hexadecene, heptadecene, octadecene, nonadecene, eicosene or mixtures thereof. In one embodiment, hexadecene, heptadecene, octadecene, nonadecene, eicosene or mixtures thereof and their dimers, trimers and tetramers are especially useful olefins. Alternatively, the olefin may be a Diels-Alder adduct of a diene such as 1,3-butadiene and an unsaturated ester, such as, butylacrylate.

Another class of sulfurized olefin includes sulfurized fatty acids and their esters. The fatty acids are often obtained from vegetable oil or animal oil and typically contain about 4 to about 22 carbon atoms. Examples of suitable fatty acids and their esters include triglycerides, oleic acid, linoleic acid, palmitoleic acid or mixtures thereof. Often, the fatty acids are obtained from lard oil, tall oil, peanut oil, soybean oil, cottonseed oil, sunflower seed oil or mixtures thereof. Fatty acids and/or ester may be mixed with olefins, such as  $\alpha$ -olefins.

In another alternative embodiment the antioxidant composition also contains a molybdenum-containing antioxidant in addition to the phenolic and/or aminic antioxidants discussed above. When a combination of these three antioxidants is used, preferably the ratio of phenolic to aminic to molybdenum-containing is (0 to 2):(0 to 2):(0 to 1).

The one or more antioxidant(s) may be present in ranges about 0 wt % to about 20 wt %, or about 0.1 wt % to about 10 wt %, or about 1 wt % to about 5 wt %, of the lubricating oil composition.

**Antiwear Agents:** The lubricating oil compositions herein also may optionally contain one or more antiwear agents. Examples of suitable additional antiwear agents include, but are not limited to, a metal thiophosphate; a metal dialkyl-dithiophosphate; a phosphoric acid ester or salt thereof, a phosphate ester(s); a phosphite; a phosphorus-containing carboxylic ester, ether, or amide; a sulfurized olefin; thiocarbamate-containing compounds including, thiocarbamate esters, alkylene-coupled thiocarbamates, and bis(S-alkyldithiocarbamyl) disulfides; and mixtures thereof. A suitable antiwear agent may be a molybdenum dithiocarbamate. The phosphorus containing antiwear agents are more fully described in European Patent 612 839. The metal in the dialkyl dithio phosphate salts may be an alkali metal, alkaline earth metal, aluminum, lead, tin, molybdenum, manganese, nickel, copper, titanium, or zinc. A useful antiwear agent may be zinc dialkyldithiophosphate.

Further examples of suitable antiwear agents include titanium compounds, tartrates, tartrimides, oil soluble amine salts of phosphorus compounds, sulfurized olefins, phosphites (such as dibutyl phosphite), phosphonates, thiocarbamate-containing compounds, such as thiocarbamate esters, thiocarbamate amides, thiocarbamic ethers, alkylene-coupled thiocarbamates, and bis(S-alkyldithiocarbamyl) disulfides. The tartrate or tartrimide may contain alkyl-ester

groups, where the sum of carbon atoms on the alkyl groups may be at least 8. The antiwear agent may in one embodiment include a citrate.

The antiwear agent may be present in ranges including about 0 wt % to about 15 wt %, or about 0.01 wt % to about 10 wt %, or about 0.05 wt % to about 5 wt %, or about 0.1 wt % to about 3 wt % of the lubricating oil composition.

**Boron-Containing Compounds:** The lubricating oil compositions herein may optionally contain one or more boron-containing compounds. Examples of boron-containing compounds include borate esters, borated fatty amines, borated epoxides, borated detergents, and borated dispersants, such as borated succinimide dispersants, as disclosed in U.S. Pat. No. 5,883,057. The boron-containing compound, if present, can be used in an amount sufficient to provide up to about 8 wt %, about 0.01 wt % to about 7 wt %, about 0.05 wt % to about 5 wt %, or about 0.1 wt % to about 3 wt % of the lubricating oil composition.

**Detergents:** The lubricating oil composition may optionally include one or more additional neutral, low based, or overbased detergents, or mixtures thereof. Suitable detergent substrates include phenates, sulfur containing phenates, sulfonates, calixarates, salixarates, salicylates, carboxylic acids, phosphorus acids, mono- and/or di-thiophosphoric acids, alkyl phenols, sulfur coupled alkyl phenol compounds, or methylene bridged phenols. Suitable detergents and their methods of preparation are described in greater detail in numerous patent publications, including U.S. Pat. No. 7,732,390 and references cited therein.

The detergent substrate may be salted with an alkali or alkaline earth metal such as, but not limited to, calcium, magnesium, potassium, sodium, lithium, barium, or mixtures thereof. In some embodiments, the detergent is free of barium. In some embodiments, a detergent may contain traces of other metals such as magnesium or calcium in amounts such as 50 ppm or less, 40 ppm or less, 30 ppm or less, 20 ppm or less, or 10 ppm or less. A suitable detergent may include alkali or alkaline earth metal salts of petroleum sulfonic acids and long chain mono- or di-alkylarylsulfonic acids with the aryl group being benzyl, tolyl, and xylol. Examples of suitable detergents include, but are not limited to, calcium phenates, calcium sulfur containing phenates, calcium sulfonates, calcium calixarates, calcium salixarates, calcium salicylates, calcium carboxylic acids, calcium phosphorus acids, calcium mono- and/or di-thiophosphoric acids, calcium alkyl phenols, calcium sulfur coupled alkyl phenol compounds, calcium methylene bridged phenols, magnesium phenates, magnesium sulfur containing phenates, magnesium sulfonates, magnesium calixarates, magnesium salixarates, magnesium salicylates, magnesium carboxylic acids, magnesium phosphorus acids, magnesium mono- and/or di-thiophosphoric acids, magnesium alkyl phenols, magnesium sulfur coupled alkyl phenol compounds, magnesium methylene bridged phenols, sodium phenates, sodium sulfur containing phenates, sodium sulfonates, sodium calixarates, sodium salixarates, sodium salicylates, sodium carboxylic acids, sodium phosphorus acids, sodium mono- and/or di-thiophosphoric acids, sodium alkyl phenols, sodium sulfur coupled alkyl phenol compounds, or sodium methylene bridged phenols.

Overbased detergent additives are well known in the art and may be alkali or alkaline earth metal overbased detergent additives. Such detergent additives may be prepared by reacting a metal oxide or metal hydroxide with a substrate and carbon dioxide gas. The substrate is typically an acid,

for example, an acid such as an aliphatic substituted sulfonic acid, an aliphatic substituted carboxylic acid, or an aliphatic substituted phenol.

An overbased detergent of the lubricating oil composition may have a total base number (TBN) of about 200 mg KOH/gram or greater, or as further examples, about 250 mg KOH/gram or greater, or about 350 mg KOH/gram or greater, or about 375 mg KOH/gram or greater, or about 400 mg KOH/gram or greater.

10 Examples of suitable overbased detergents include, but are not limited to, overbased calcium phenates, overbased calcium sulfur containing phenates, overbased calcium sulfonates, overbased calcium calixarates, overbased calcium salixarates, overbased calcium salicylates, overbased calcium carboxylic acids, overbased calcium phosphorus acids, overbased calcium mono- and/or di-thiophosphoric acids, overbased calcium alkyl phenols, overbased calcium sulfur coupled alkyl phenol compounds, overbased magnesium phenates, overbased magnesium sulfur containing phenates, overbased magnesium sulfonates, overbased magnesium calixarates, overbased magnesium salixarates, overbased magnesium salicylates, overbased magnesium carboxylic acids, overbased magnesium phosphorus acids, overbased magnesium mono- and/or di-thiophosphoric acids, overbased magnesium alkyl phenols, overbased magnesium sulfur coupled alkyl phenol compounds, or overbased magnesium methylene bridged phenols.

The overbased calcium phenate detergents have a total base number of at least about 150 mg KOH/g, at least about 225 mg KOH/g, at least about 225 mg KOH/g to about 400 mg KOH/g, at least about 225 mg KOH/g to about 350 mg KOH/g or about 230 mg KOH/g to about 350 mg KOH/g, all as measured by the method of ASTM D-2896. When such detergents are formed in an inert diluent, e.g. a process oil, usually a mineral oil, the total base number reflects the basicity of the overall composition including diluent, and any other materials (e.g., promoter, etc.) that may be contained in the detergent composition.

40 The overbased detergent may have a metal to substrate ratio of from 1.1:1, or from 2:1, or from 4:1, or from 5:1, or from 7:1, or from 10:1. In some embodiments, a detergent is effective at reducing or preventing rust in an engine or other automotive part such as a transmission or gear. The detergent may be present in a lubricating composition at about 0 wt % to about 10 wt %, or about 0.1 wt % to about 8 wt %, or about 1 wt % to about 4 wt %, or greater than about 4 wt % to about 8 wt %.

**Extreme Pressure Agents:** The lubricating oil compositions herein may optionally contain one or more extreme pressure agents. Extreme Pressure (EP) agents that are soluble in the oil include sulfur- and chlorosulfur-containing EP agents, chlorinated hydrocarbon EP agents and phosphorus EP agents. Examples of such EP agents include chlorinated wax; organic sulfides and polysulfides such as dibenzylidisulfide, bis(chlorobenzyl) disulfide, dibutyl tetrasulfide, sulfurized methyl ester of oleic acid, sulfurized alkyl phenol, sulfurized dipentene, sulfurized terpene, and sulfurized Diels-Alder adducts; phosphorusulfurized hydrocarbons such as the reaction product of phosphorus sulfide with turpentine or methyl oleate; phosphorus esters such as the dihydrocarbyl and trihydrocarbyl phosphites, e.g., dibutyl phosphite, diheptyl phosphite, dicyclohexyl phosphite, pentylphenyl phosphite; diphenylphenyl phosphite, tridecyl phosphite, distearyl phosphite and polypropylene substituted phenyl phosphite; metal thiocarbamates such as zinc diocetylthiocarbamate and barium heptylphenol diacid; amine salts of alkyl

and dialkylphosphoric acids, including, for example, the amine salt of the reaction product of a dialkyldithiophosphoric acid with propylene oxide; and mixtures thereof.

**Friction Modifiers:** The lubricating oil compositions herein may optionally contain one or more friction modifiers. Suitable friction modifiers may comprise metal containing and metal-free friction modifiers and may include, but are not limited to, imidazolines, amides, amines, succinimides, alkoxylated amines, alkoxylated ether amines, amine oxides, amidoamines, nitriles, betaines, quaternary amines, imines, amine salts, amino guanadine, alkanolamides, phosphonates, metal-containing compounds, glycerol esters, sulfurized fatty compounds and olefins, sunflower oil other naturally occurring plant or animal oils, dicarboxylic acid esters, esters or partial esters of a polyol and one or more aliphatic or aromatic carboxylic acids, and the like.

Suitable friction modifiers may contain hydrocarbyl groups that are selected from straight chain, branched chain, or aromatic hydrocarbyl groups or mixtures thereof, and may be saturated or unsaturated. The hydrocarbyl groups may be composed of carbon and hydrogen or hetero atoms such as sulfur or oxygen. The hydrocarbyl groups may range from about 12 to about 25 carbon atoms. In some embodiments the friction modifier may be a long chain fatty acid ester. In another embodiment the long chain fatty acid ester may be a mono-ester, or a di-ester, or a (tri)glyceride. The friction modifier may be a long chain fatty amide, a long chain fatty ester, a long chain fatty epoxide derivatives, or a long chain imidazoline.

Other suitable friction modifiers may include organic, ashless (metal-free), nitrogen-free organic friction modifiers. Such friction modifiers may include esters formed by reacting carboxylic acids and anhydrides with alkanols and generally include a polar terminal group (e.g. carboxyl or hydroxyl) covalently bonded to an oleophilic hydrocarbon chain. An example of an organic ashless nitrogen-free friction modifier is known generally as glycerol monooleate (GMO) which may contain mono-, di-, and tri-esters of oleic acid. Other suitable friction modifiers are described in U.S. Pat. No. 6,723,685, herein incorporated by reference in its entirety.

Aminic friction modifiers may include amines or polyamines. Such compounds can have hydrocarbyl groups that are linear, either saturated or unsaturated, or a mixture thereof and may contain from about 12 to about 25 carbon atoms. Further examples of suitable friction modifiers include alkoxylated amines and alkoxylated ether amines. Such compounds may have hydrocarbyl groups that are linear, either saturated, unsaturated, or a mixture thereof. They may contain from about 12 to about 25 carbon atoms. Examples include ethoxylated amines and ethoxylated ether amines.

The amines and amides may be used as such or in the form of an adduct or reaction product with a boron compound such as a boric oxide, boron halide, metaborate, boric acid or a mono-, di- or tri-alkyl borate. Other suitable friction modifiers are described in U.S. Pat. No. 6,300,291, herein incorporated by reference in its entirety.

A friction modifier may optionally be present in ranges such as about 0 wt % to about 10 wt %, or about 0.01 wt % to about 8 wt %, or about 0.1 wt % to about 4 wt %.

**Molybdenum-containing component:** The lubricating oil compositions herein may optionally contain one or more molybdenum-containing compounds. An oil-soluble molybdenum compound may have the functional performance of an antiwear agent, an antioxidant, a friction modifier, or mixtures thereof. An oil-soluble molybdenum compound

may include molybdenum dithiocarbamates, molybdenum dialkyldithiophosphates, molybdenum dithiophosphinates, amine salts of molybdenum compounds, molybdenum xanthates, molybdenum thioxanthates, molybdenum sulfides, molybdenum carboxylates, molybdenum alkoxides, a tri-nuclear organo-molybdenum compound, and/or mixtures thereof. The molybdenum sulfides include molybdenum disulfide. The molybdenum disulfide may be in the form of a stable dispersion. In one embodiment the oil-soluble molybdenum compound may be selected from the group consisting of molybdenum dithiocarbamates, molybdenum dialkyldithiophosphates, amine salts of molybdenum compounds, and mixtures thereof. In one embodiment the oil-soluble molybdenum compound may be a molybdenum dithiocarbamate.

Suitable examples of molybdenum compounds which may be used include commercial materials sold under the trade names such as Molyvan® 822™, Molyvan® A, 20 Molyvan® 2000 and Molyvan® 855, and Molyvan® 1055 from R. T. Vanderbilt Co., Ltd., and Sakura-Lube™ S-165, S-200, S-300, S-310G, S-151, S-525, S-600, S-700, and S-710 available from Adeka Corporation, and mixtures thereof. Suitable molybdenum components are described in 25 U.S. Pat. No. 5,650,381; US RE 37,363 E1; US RE 38,929 E1; and US RE 40,595 E1, incorporated herein by reference in their entireties.

Additionally, the molybdenum compound may be an acidic molybdenum compound. Included are molybdic acid, ammonium molybdate, sodium molybdate, potassium molybdate, and other alkaline metal molybdates and other molybdenum salts, e.g., hydrogen sodium molybdate, MoOCl<sub>4</sub>, MoO<sub>2</sub>Br<sub>2</sub>, Mo<sub>2</sub>03C<sub>16</sub>, molybdenum trioxide or similar acidic molybdenum compounds. Alternatively, the compositions can be provided with molybdenum by molybdenum/sulfur complexes of basic nitrogen compounds as described, for example, in U.S. Pat. Nos. 4,263,152; 4,285, 822; 4,283,295; 4,272,387; 4,265,773; 4,261,843; 4,259,195 and 4,259,194; and WO 94/06897, incorporated herein by reference in their entireties.

Another class of suitable organo-molybdenum compounds are tri-nuclear molybdenum compounds, such as those of the formula Mo<sub>3</sub>SkLnQz and mixtures thereof, 45 wherein S represents sulfur, L represents independently selected ligands having organo groups with a sufficient number of carbon atoms to render the compound soluble or dispersible in the oil, n is from 1 to 4, k varies from 4 through 7, Q is selected from the group of neutral electron 50 donating compounds such as water, amines, alcohols, phosphines, and ethers, and z ranges from 0 to 5 and includes non-stoichiometric values. At least 21 total carbon atoms may be present among all the ligands' organo groups, such as at least 25, at least 30, or at least 35 carbon atoms. 55 Additional suitable molybdenum compounds are described in U.S. Pat. No. 6,723,685, herein incorporated by reference in its entirety.

The oil-soluble molybdenum compound may be present in an amount sufficient to provide about 0.5 ppm to about 60 2000 ppm, about 1 ppm to about 700 ppm, about 1 ppm to about 550 ppm, about 5 ppm to about 300 ppm, or about 20 ppm to about 250 ppm of molybdenum.

**Transition Metal-containing compounds:** In another embodiment, the lubricants herein may optionally include a transition metal containing compound or a metalloid. The transition metals may include, but are not limited to, titanium, vanadium, copper, zinc, zirconium, molybdenum,

21

tantalum, tungsten, and the like. Suitable metalloids include, but are not limited to, boron, silicon, antimony, tellurium, and the like.

In an embodiment, an oil-soluble transition metal-containing compound may function as antiwear agents, friction modifiers, antioxidants, deposit control additives, or more than one of these functions. In an embodiment the oil-soluble transition metal-containing compound may be an oil-soluble titanium compound, such as a titanium (IV) alkoxide. Among the titanium containing compounds that may be used in, or which may be used for preparation of the oil-soluble materials of, the disclosed technology are various Ti (IV) compounds such as titanium (IV) oxide; titanium (IV) sulfide; titanium (IV) nitrate; titanium (IV) alkoxides such as titanium methoxide, titanium ethoxide, titanium propoxide, titanium isopropoxide, titanium butoxide, titanium 2-ethylhexoxide; and other titanium compounds or complexes including but not limited to titanium phenates; titanium carboxylates such as titanium (IV) 2-ethyl-1-3-hexanedioate or titanium citrate or titanium oleate; and titanium (IV) (triethanolaminato)isopropoxide. Other forms of titanium encompassed within the disclosed technology include titanium phosphates such as titanium dithiophosphates (e.g., dialkyldithiophosphates) and titanium sulfonates (e.g., alkylbenzenesulfonates), or, generally, the reaction product of titanium compounds with various acid materials to form salts, such as oil-soluble salts. Titanium compounds can thus be derived from, among others, organic acids, alcohols, and glycols. Ti compounds may also exist in dimeric or oligomeric form, containing Ti—O—Ti structures. Such titanium materials are commercially available or can be readily prepared by appropriate synthesis techniques which will be apparent to the person skilled in the art. They may exist at room temperature as a solid or a liquid, depending on the particular compound. They may also be provided in a solution form in an appropriate inert solvent.

In one embodiment, the titanium can be supplied as a Ti-modified dispersant, such as a succinimide dispersant. Such materials may be prepared by forming a titanium mixed anhydride between a titanium alkoxide and a hydrocarbyl-substituted succinic anhydride, such as an alkenyl- (or alkyl) succinic anhydride. The resulting titanate-succinate intermediate may be used directly or it may be reacted with any of a number of materials, such as (a) a polyamine-based succinimide/amide dispersant having free, condensable —NH functionality; (b) the components of a polyamine-based succinimide/amide dispersant, i.e., an alkenyl- (or alkyl-) succinic anhydride and a polyamine, (c) a hydroxy-containing polyester dispersant prepared by the reaction of a substituted succinic anhydride with a polyol, aminoalcohol, polyamine, or mixtures thereof. Alternatively, the titanate-succinate intermediate may be reacted with other agents such as alcohols, aminoalcohols, ether alcohols, polyether alcohols or polyols, or fatty acids, and the product thereof either used directly to impart Ti to a lubricant, or else further reacted with the succinic dispersants as described above. As an example, 1 part (by mole) of tetraisopropyl titanate may be reacted with about 2 parts (by mole) of a polyisobutene-substituted succinic anhydride at 140-150° C. for 5 to 6 hours to provide a titanium modified dispersant or intermediate. The resulting material (30 g) may be further reacted with a succinimide dispersant from polyisobutene-substituted succinic anhydride and a polyethylenepolyamine mixture (127 grams+diluent oil) at 150° C. for 1.5 hours, to produce a titanium-modified succinimide dispersant.

22

Another titanium containing compound may be a reaction product of titanium alkoxide and C<sub>6</sub> to C<sub>25</sub> carboxylic acid. The reaction product may be represented by the following formula:



wherein n is an integer selected from 2, 3 and 4, and R is a hydrocarbyl group containing from about 5 to about 24 carbon atoms, or by the formula:



wherein  $m+n=4$  and  $n$  ranges from 1 to 3,  $R_4$  is an alkyl moiety with carbon atoms ranging from 1-8,  $R_1$  is selected from a hydrocarbyl group containing from about 6 to 25 carbon atoms, and  $R_2$  and  $R_3$  are the same or different and are selected from a hydrocarbyl group containing from about 1 to 6 carbon atoms, or the titanium compound may be represented by the formula:



wherein x ranges from 0 to 3,  $R_1$  is selected from a hydrocarbyl group containing from about 6 to 25 carbon atoms,  $R_2$ , and  $R_3$  are the same or different and are selected from a hydrocarbyl group containing from about 1 to 6 carbon atoms, and  $R_4$  is selected from a group consisting of either H, or  $C_6$  to  $C_{25}$  carboxylic acid moiety.

Suitable carboxylic acids may include, but are not limited to caproic acid, caprylic acid, lauric acid, myristic acid, palmitic acid, stearic acid, arachidic acid, oleic acid, erucic acid, linoleic acid, linolenic acid, cyclohexanecarboxylic acid, phenylacetic acid, benzoic acid, neodecanoic acid, and the like.

In an embodiment the oil soluble titanium compound may be present in the lubricating oil composition in an amount to provide from 0 to 3000 ppm titanium by weight or 25 to about 1500 ppm titanium by weight or about 35 ppm to 500 ppm titanium by weight or about 50 ppm to about 300 ppm.

Viscosity Index Improvers: The lubricating oil compositions herein may optionally contain one or more viscosity index improvers. Suitable viscosity index improvers may include polyolefins, olefin copolymers, ethylene/propylene

copolymers, polyisobutenes, hydrogenated styrene-isoprene polymers, styrene/maleic ester copolymers, hydrogenated styrene/butadiene copolymers, hydrogenated isoprene polymers, alpha-olefin maleic anhydride copolymers, polymethacrylates, polyacrylates, polyalkyl styrenes, hydrogenated alkenyl aryl conjugated diene copolymers, or mixtures thereof. Viscosity index improvers may include star polymers and suitable examples are described in US Publication No. 20120101017A1.

The lubricating oil compositions herein may optionally contain one or more dispersant viscosity index improvers in addition to a viscosity index improver or in lieu of a viscosity index improver. Suitable viscosity index improvers may include functionalized polyolefins, for example, ethylene-propylene copolymers that have been functionalized with the reaction product of an acylating agent (such as maleic anhydride) and an amine; polymethacrylates functionalized with an amine, or esterified maleic anhydride-styrene copolymers reacted with an amine.

The total amount of viscosity index improver and/or dispersant viscosity index improver may be about 0 wt % to about 20 wt %, about 0.1 wt % to about 15 wt %, about 0.1 wt % to about 12 wt %, or about 0.5 wt % to about 10 wt %, of the lubricating oil composition.

Other Optional Additives: Other additives may be selected to perform one or more functions required of a lubricating fluid. Further, one or more of the mentioned additives may be multi-functional and provide functions in addition to or other than the function prescribed herein. The other performance additives may be in addition to specified additives of the present disclosure and/or may comprise one or more of metal deactivators, viscosity index improvers, detergents, ashless TBN boosters, friction modifiers, anti-wear agents, corrosion inhibitors, rust inhibitors, dispersants, dispersant viscosity index improvers, extreme pressure agents, antioxidants, foam inhibitors, demulsifiers, emulsifiers, pour point depressants, seal swelling agents and mixtures thereof. Typically, fully-formulated lubricating oil will contain one or more of these performance additives.

Suitable metal deactivators may include derivatives of benzotriazoles (typically tolyltriazole), dimercaptothiadiazoles derivatives, 1,2,4-triazoles, benzimidazoles, 2-alkyldithiobenzimidazoles, or 2-alkyldithiobenzothiazoles; foam inhibitors including copolymers of ethyl acrylate and 2-ethylhexylacrylate and optionally vinyl acetate; demulsifiers

including trialkyl phosphates, polyethylene glycols, polyethylene oxides, polypropylene oxides and (ethylene oxide-propylene oxide) polymers; pour point depressants including esters of maleic anhydride-styrene, polymethacrylates, polyacrylates or polyacrylamides.

Suitable foam inhibitors include silicon-based compounds, such as siloxane.

Suitable pour point depressants may include a polymethacrylates or mixtures thereof. Pour point depressants may be present in an amount sufficient to provide from about 0 wt % to about 1 wt %, about 0.01 wt % to about 0.5 wt %, or about 0.02 wt % to about 0.04 wt % based upon the final weight of the lubricating oil composition.

Suitable additional rust inhibitors may be a single compound or a mixture of compounds having the property of inhibiting corrosion of ferrous metal surfaces. Additional rust inhibitors may be provided so long as they do not conflict with the selected corrosion inhibitors discussed above. Non-limiting examples of rust inhibitors, in addition to those described above, include oil-soluble high molecular weight organic acids, such as 2-ethylhexanoic acid, lauric acid, myristic acid, palmitic acid, oleic acid, linoleic acid, linolenic acid, behenic acid, and cerotic acid, as well as oil-soluble polycarboxylic acids including dimer and trimer acids, such as those produced from tall oil fatty acids, oleic acid, and linoleic acid. Other suitable corrosion inhibitors include long-chain alpha, omega-dicarboxylic acids in the molecular weight range of about 600 to about 3000 and alkenylsuccinic acids in which the alkenyl group contains about 10 or more carbon atoms such as, tetrapropenylsuccinic acid, tetradecenylsuccinic acid, and hexadecenylsuccinic acid. Another useful type of acidic corrosion inhibitors are the half esters of alkenyl succinic acids having about 8 to about 24 carbon atoms in the alkenyl group with alcohols such as the polyglycols. The corresponding half amides of such alkenyl succinic acids are also useful. A useful rust inhibitor is a high molecular weight organic acid.

The rust inhibitor, if present, can be used in an amount sufficient to provide about 0 wt % to about 5 wt %, about 0.01 wt % to about 3 wt %, about 0.1 wt % to about 2 wt %, based upon the final weight of the lubricating oil composition.

In general terms, a suitable lubricant including the low levels of sulfated ash and the select acyclic rust or corrosion inhibitors herein may include additive components in the ranges listed in the following table.

TABLE 2

| Suitable Low-Ash Lubricating Compositions |                                 |                                 |
|-------------------------------------------|---------------------------------|---------------------------------|
| Component                                 | Wt. %<br>(Suitable Embodiments) | Wt. %<br>(Suitable Embodiments) |
| Acyclic corrosion inhibitor(s)            | 0.02-0.3                        | 0.03-0.2                        |
| Succinimide Dispersant(s)                 | 1.0-8.0                         | 2.5-5.5                         |
| Antioxidant(s)                            | 0.3-4.0                         | 0.5-3.0                         |
| Detergent(s)                              | 0.5-4.0                         | 0.75-3.0                        |
| Antiwear (ZDDP)                           | 0.1-2.0                         | 0.5-1.5                         |
| Ashless TBN booster(s)                    | 0.0-1.0                         | 0.01-0.5                        |
| Other Corrosion inhibitor(s)              | 0.0-5.0                         | 0.0-2.0                         |
| Metal dihydrocarbyldithiophosphate(s)     | 0.0-6.0                         | 0.1-4.0                         |
| Ash-free phosphorus compound(s)           | 0.0-6.0                         | 0.0-4.0                         |
| Antifoaming agent(s)                      | 0.0-5.0                         | 0.001-0.15                      |
| Antiwear agent(s)                         | 0.0-1.0                         | 0.0-0.8                         |
| Pour point depressant(s)                  | 0.0-5.0                         | 0.01-1.5                        |
| Viscosity index improver(s)               | 0.0-25.0                        | 0.1-15.0                        |
| Dispersant viscosity index improver(s)    | 0.0-10.0                        | 0.0-5.0                         |
| Friction modifier(s)                      | 0.0-5.0                         | 0.01-2.0                        |
| Base oil                                  | Balance                         | Balance                         |
| Total                                     | 100                             | 100                             |

The percentages of each component above represent the weight percent of each component, based upon the weight of the final lubricating oil composition. The remainder of the lubricating oil composition consists of one or more base oils. Additives used in formulating the compositions described herein may be blended into the base oil individually or in various sub-combinations. However, it may be suitable to blend all of the components concurrently using an additive concentrate (i.e., additives plus a diluent, such as a hydrocarbon solvent). Fully formulated lubricants conventionally contain an additive package, referred to herein as a dispersant/inhibitor package or DI package, that will supply the characteristics that are required in the formulation.

Lubricants herein are configured for use in various types of lubricants, such as automotive lubricants and/or greases, internal combustion engine oils, hybrid engine oils, electric engine lubricants, drivetrain lubricants, transmission lubricants, gear oils, hydraulic lubricants, tractor hydraulic fluids, metal working fluids, turbine engine lubricants, stationary engine lubricants, tractor lubricants, motorcycle lubricants, power steering fluids, clutch fluids, axles fluids, wet break fluids, and the like. Suitable engine types may include, but are not limited to heavy-duty diesel, passenger car, light duty diesel, medium speed diesel, or marine engines. An internal combustion engine may be a diesel fueled engine, a gasoline fueled engine, a natural gas fueled engine, a bio-fueled engine, a mixed diesel/biofuel fueled engine, a mixed gasoline/biofuel fueled engine, an alcohol fueled engine, a mixed gasoline/alcohol fueled engine, a compressed natural gas (CNG) fueled engine, or mixtures thereof. A diesel engine may be a compression-ignited engine. A gasoline engine may be a spark-ignited engine. An internal combustion engine may also be used in combination with an electrical or battery source of power. An engine so configured is commonly known as a hybrid engine. The internal combustion engine may be a 2-stroke, 4-stroke, or rotary engine. Suitable internal combustion engines include marine diesel engines (such as inland marine), aviation piston engines, low-load diesel engines, and motorcycle, automobile, locomotive, and truck engines. Engines may be coupled with a turbocharger.

The lubricating oil composition for an internal combustion engine may be suitable for any engine lubricant irrespective of the sulfur, phosphorus, or ash calculated as sulfated ash (ASTM D-874) content. The sulfur content of the engine oil lubricant may be about 1 wt % or less, or about 0.8 wt % or less, or about 0.5 wt % or less, or about 0.3 wt % or less, or about 0.2 wt % or less. In one embodiment the sulfur content may be in the range of about 0.001 wt % to about 0.5 wt %, or about 0.01 wt % to about 0.3 wt %. The phosphorus content may be about 0.2 wt % or less, or about 0.1 wt % or less, or about 0.085 wt % or less, or about 0.08 wt % or less, or even about 0.06 wt % or less, about 0.055 wt % or less, or about 0.05 wt % or less. In one embodiment, the phosphorus content may be about 50 ppm to about 1000 ppm, or about 325 ppm to about 850 ppm. The total sulfated ash content may be about 2 wt % or less, or about 1.5 wt % or less, or about 1.1 wt % or less, or about 1 wt % or less, or about 0.8 wt % or less, or about 0.5 wt % or less. In one embodiment the sulfated ash content may be about 0.05 wt % to about 0.9 wt %, or about 0.1 wt % or about 0.2 wt % to about 0.45 wt %. In another embodiment, the sulfur content may be about 0.4 wt % or less, the phosphorus content may be about 0.08 wt % or less, and the sulfated ash is about 1 wt % or less. In yet another embodiment the sulfur

content may be about 0.3 wt % or less, the phosphorus content is about 0.05 wt % or less, and the sulfated ash may be about 0.8 wt % or less.

Further, lubricants of the present description may be suitable to meet one or more industry specification requirements such as IL-SAC GF-3, GF-4, GF-5, GF-6, PC-11, CF, CF-4, CH-4, CK-4, FA-4, CJ-4, CI-4 Plus, CI-4, API SG, SJ, SL, SM, SN, SN PLUS, ACEA A1/B1, A2/B2, A3/B3, A3/B4, A5/B5, A7/B7, C1, C2, C3, C4, C5, C6, E4/E6/E7/E9, Euro 5/6, JASO DL-1, Low SAPS, Mid SAPS, or original equipment manufacturer specifications such as Dexos1™, Dexos2™, MB-Approval 229.1, 229.3, 229.5, 229.51/229.31, 229.52, 229.6, 229.71, 226.5, 226.51, 228.0/0.1, 228.2/0.3, 228.31, 228.5, 228.51, 228.61, VW 501.01, 502.00, 503.00/503.01, 504.00, 505.00, 505.01, 506.00/0.1, 507.00, 508.00, 509.00, 508.88, 509.99, BMW Longlife-01, Longlife-01 FE, Longlife-04, Longlife-12 FE, Longlife-14 FE+, Longlife-17 FE+, Porsche A40, C30, Peugeot Citroen Automobiles B71 2290, B71 2294, B71 2295, B71 2296, B71 2297, B71 2300, B71 2302, B71 2312, B71 2007, B71 2008, Renault RN0700, RN0710, RN0720, Ford WSS-M2C153-H, WSS-M2C930-A, WSS-M2C945-A, WSS-M2C913A, WSS-M2C913-B, WSS-M2C913-C, WSS-M2C913-D, WSS-M2C948-B, WSS-M2C948-A, GM 6094-M, Chrysler MS-6395, Fiat 9.55535 G1, G2, M2, N1, N2, Z2, S1, S2, S3, S4, T2, DS1, DSX, GH2, GS1, GSX, CR1, Jaguar Land Rover STJLR.03.5003, STJLR.03.5004, STJLR.03.5005, STJLR.03.5006, STJLR.03.5007, STJLR.51.5122 or any past or future PCMO or HDD specifications not mentioned herein. In some embodiments for passenger car motor oil (PCMO) applications, the amount of phosphorus in the finished fluid is 1000 ppm or less or 900 ppm or less or 800 ppm or less.

In one embodiment, the lubricating oil composition is an engine oil, wherein the lubricating oil composition may have (i) a sulfur content of about 0.5 wt % or less, (ii) a phosphorus content of about 0.1 wt % or less, and (iii) ash calculated as sulfated ash content of about 1.5 wt % or less.

In one embodiment, the lubricating oil composition is suitable for a 2-stroke or a 4-stroke marine diesel internal combustion engine. In one embodiment, the marine diesel combustion engine is a 2-stroke engine. In some embodiments, the lubricating oil composition is not suitable for a 2-stroke or a 4-stroke marine diesel internal combustion engine for one or more reasons, including but not limited to, the high sulfur content of fuel used in powering a marine engine and the high TBN required for a marine-suitable engine oil (e.g., above about 40 TBN in a marine-suitable engine oil).

In some embodiments, the lubricating oil composition is suitable for use with engines powered by low sulfur fuels, such as fuels containing about 1 to about 5% sulfur. Highway vehicle fuels contain about 15 ppm sulfur (or about 0.0015% sulfur).

## EXAMPLES

The following examples are illustrative of exemplary embodiments of the disclosure. In these examples, as well as elsewhere in this application, all ratios, parts, and percentages are by weight unless otherwise indicated. It is intended that these examples are being presented for the purpose of illustration only and are not intended to limit the scope of the invention disclosed herein.

### Comparative Example 1

A Comparative Lubricating Composition CE1 having a sulfated ash content of about 0.7 weight percent had the

analytics of Table 3 below and included a standard additive package of dispersant(s), detergent(s), antiwear additive(s), antioxidant(s), organo-molybdenum additive(s), antifoam additive(s), friction modifier(s), olefin copolymer viscosity modifier(s), pour point dispersant(s), process oil(s) and base oil(s) to provide a finished lubricant having a KV100 of about 7.0 cSt (ASTM D445).

TABLE 3

|                     |        |      |
|---------------------|--------|------|
| KV100               | cSt    | 6.9  |
| Boron               | ppm    | 59   |
| Ca                  | ppm    | 1392 |
| Mg                  | ppm    | 371  |
| Mo                  | ppm    | 50   |
| Na                  | ppm    | 0    |
| P                   | ppm    | 634  |
| Zinc                | ppm    | 693  |
| TBN (D2896)         | mg KOH | 7.3  |
| TBN (D4739)         | mg KOH | 5.4  |
| Sulfated ash (D874) | %      | 0.67 |

The calculated sulfated ash (SASH) for Table 3 above was determined pursuant to ASTM D874. The Comparative Lubricating Composition CE1 of this Example did not include any corrosion inhibitors and, thus, failed the engine oil moisture test pursuant to GMW 16073 with a corrosion rating of 4 reflecting a strong level of corrosion. As set forth in GMW 16073, a corrosion rating of 0 means no corrosion, a rating of 1 means trace corrosion with a maximum of 5 corrosion spots (with maximum diameter of each spot being 1 mm), a rating of 2 means slight corrosion with corrosion up to about 5 percent of the surface, a rating of 3 means medium corrosion with corrosion between 5 percent to 20 percent of the surface, and a rating of 4 means strong corrosion with corrosion on more than 20 percent of the surface.

#### Comparative Example 2

Another Comparative Lubricant CE2 was evaluated for steel corrosion when the additive package was reformulated to provide sulfated ash levels below 0.1 weight percent.

Table 4 below shows the analytics of Comparative Lubricant CE2 with a base additive package that included dispersant(s), antiwear additive(s), antioxidant(s), organo-molybdenum additive(s), antifoam additive(s), friction modifies(s), olefin copolymer viscosity modifier(s), pour point dispersant(s), process oil(s) and base oil(s) to form a finished lubricant having an extreme low ash content of about 0.1 percent or less and having a KV100 of about 9.5 cSt.

TABLE 4

|                     |        |      |
|---------------------|--------|------|
| KV100               | cSt    | 9.5  |
| Boron               | ppm    | 58   |
| Calcium             | ppm    | 6    |
| Magnesium           | ppm    | 2    |
| Molybdenum          | ppm    | 0    |
| Sodium              | ppm    | 0    |
| Phosphorus          | ppm    | 190  |
| Zinc                | ppm    | 0    |
| TBN (D2896)         | mg KOH | 4.3  |
| TBN (D4739)         | mg KOH | 0.7  |
| Sulfated ash (D874) | %      | 0.06 |

The Comparative Lubricant CE2 also did not include any corrosion inhibitors and, thus, still failed the engine oil moisture testing performed pursuant to GMW 16073 with slight corrosion having a corrosion rating of 2, but with the extreme low ash content, the Comparative Lubricant CE2 also failed the high temperature deposit formation test of ASTM D6335 (TEOST-33C) with 33.4 mg of high temperature deposits (less than 30 mg is preferred).

#### Example 1

Various corrosion inhibitor chemistries were investigated as a top treat in the extreme low ash lubricant formulation of Comparative Example 2. Lubricants of this Example included the same additive package and base oil blend of lubricant CE2 to achieve a sulfated ash content of about 0.06%, but were combined with different amounts of varying corrosion inhibitor chemistries as described in Table 5 below.

TABLE 5

| Corrosion Inhibitor Chemistries |                                                                                                                                                        |                                              |
|---------------------------------|--------------------------------------------------------------------------------------------------------------------------------------------------------|----------------------------------------------|
|                                 | Compound                                                                                                                                               | Chemistry                                    |
| A                               | Reaction product of dodecyl succinic anhydride/acid (DDSA) with propylene glycol forming a blend of C10-C12 dicarboxylic acids and C10-C12 acid-esters | Oil soluble diacid and acid-ester blend      |
| B                               | 1-oleyl-w-(2-dihydroxyethyl)-imidazoline                                                                                                               | Oil soluble amidine                          |
| C                               | Condensation product of dodecyl succinic acid or anhydride                                                                                             | Oil soluble nitrogen free polyhydric alcohol |
| D                               | Pentaerythritol mono-oleate                                                                                                                            | Oil soluble nitrogen free polyhydric alcohol |
| E                               | Reaction product of C20-C24 alkene with succinic acid/anhydride                                                                                        | Oil soluble imide                            |
| F                               | C10-C20 fatty amide                                                                                                                                    | Oil soluble fatty amide                      |
| G                               | N,N-dialkanol fatty amine                                                                                                                              | Oil soluble polyhydroxyamine                 |

The corrosion inhibitors of Table 5 were included in finished lubricants at the treat rates of Tables 5a and 5b as a top treat to the lubricant of Comparative Example 2. The lubricants of this Example were then evaluated for steel corrosion rating (GMW 16073), emulsion stability (ASTM D7563), and high temperature deposits (ASTM D6335). The results are also provided in Tables 5a or 5b. Passing steel corrosion rating is 0 reflecting no corrosion, passing emulsion stability is 0% water separation at either 0° C. or 25° C., and passing high temperature deposits is 30 mg or less. Failing lubricants are shown by the bold and underlined cells in Tables 5a or 5b.

TABLE 5a

|                     | A    |      |      |      | B         |             |             |             | C        |      |      |           | D        |      |      |      |
|---------------------|------|------|------|------|-----------|-------------|-------------|-------------|----------|------|------|-----------|----------|------|------|------|
| Treat Rate (wt %)   | 0.02 | 0.05 | 0.18 | 0.3  | 0.02      | 0.05        | 0.18        | 0.3         | 0.02     | 0.05 | 0.18 | 0.3       | 0.02     | 0.05 | 0.18 | 0.3  |
| Total Deposit (mg)  | 6.0  | 12.6 | 13.9 | 9.9  | 25.0      | 16.8        | 19.1        | 18.6        | 19.2     | 6.9  | 11.9 | 15.7      | 12.0     | 20.6 | 14.6 | 15.6 |
| Corrosion Rating    | 0    | 0    | 0    | 0    | <b>1</b>  | 0           | 0           | <b>1</b>    | <b>1</b> | 0    | 0    | 0         | <b>1</b> | 0    | 0    | 0    |
| E85 Emulsion 25° C. | Pass | Pass | Pass | Pass | Pass      | <b>Fail</b> | <b>Fail</b> | <b>Fail</b> | Pass     | Pass | Pass | Pass      | Pass     | Pass | Pass | Pass |
| E85 Emulsion 0° C.  | Pass | Pass | Pass | Pass | Pass      | <b>Fail</b> | <b>Fail</b> | Pass        | Pass     | Pass | Pass | Pass      | Pass     | Pass | Pass | Pass |
| Inventive           | Yes  | Yes  | Yes  | Yes  | <u>No</u> | <u>No</u>   | <u>No</u>   | <u>No</u>   | Yes      | Yes  | Yes  | <u>No</u> | Yes      | Yes  | Yes  | Yes  |

TABLE 5b

|                     | E         |           |           |           | F    |      |      |      | G    |      |      |             |
|---------------------|-----------|-----------|-----------|-----------|------|------|------|------|------|------|------|-------------|
| Treat Rate (wt %)   | 0.02      | 0.05      | 0.18      | 0.3       | 0.02 | 0.05 | 0.18 | 0.3  | 0.02 | 0.05 | 0.18 | 0.3         |
| Total Deposits (mg) | 21.2      | 16.6      | 13.3      | 14.8      | 20.3 | 19.4 | 15.4 | 137  | 5.1  | 18.6 | 15.2 | 16.1        |
| Corrosion Rating    | <b>1</b>  | <b>2</b>  | <b>2</b>  | <b>1</b>  | 0    | 0    | 0    | 0    | 0    | 0    | 0    | 0           |
| E85 Emulsion 25° C. | Pass      | Pass      | Pass      | Pass      | Pass | Pass | Pass | Pass | Pass | Pass | Pass | <b>Fail</b> |
| E85 Emulsion 0° C.  | Pass      | Pass      | Pass      | Pass      | Pass | Pass | Pass | Pass | Pass | Pass | Pass | <b>Fail</b> |
| Inventive           | <u>No</u> | <u>No</u> | <u>No</u> | <u>No</u> | Yes  | Yes  | Yes  | Yes  | Yes  | Yes  | Yes  | <u>No</u>   |

As shown in Tables 5a and 5b, only certain corrosion inhibitor chemistries and only select treat rates of specific chemistries achieve passing high temperature deposits of 30 mg or less, a passing steel corrosion rating of 0, and passing E85 emulsion stability with 0 percent water separation when the lubricants are configured as extremely low sulfated ash formulations with ash levels of 0.5 weight percent or below, 0.3 weight percent or below, or 0.1 weight percent or below. It was unexpected that certain corrosion inhibitory chemistry would provide passing performance in such testing as all inhibitors generally included acidic, hydroxy, and/or nitro-  
gen-based chemistry.

It is noted that, as used in this specification and the appended claims, the singular forms "a," "an," and "the," include plural referents unless expressly and unequivocally limited to one referent. Thus, for example, reference to "an antioxidant" includes two or more different antioxidants. As used herein, the term "include" and its grammatical variants

are intended to be non-limiting, such that recitation of items in a list is not to the exclusion of other like items that can be substituted or added to the listed items

For the purposes of this specification and appended claims, unless otherwise indicated, all numbers expressing quantities, percentages or proportions, and other numerical values used in the specification and claims, are to be understood as being modified in all instances by the term "about." Accordingly, unless indicated to the contrary, the numerical parameters set forth in the following specification and attached claims are approximations that can vary depending upon the desired properties sought to be obtained by the present disclosure. At the very least, and not as an attempt to limit the application of the doctrine of equivalents to the scope of the claims, each numerical parameter should at least be construed in light of the number of reported significant digits and by applying ordinary rounding techniques.

## 31

It is to be understood that each component, compound, substituent or parameter disclosed herein is to be interpreted as being disclosed for use alone or in combination with one or more of each and every other component, compound, substituent or parameter disclosed herein.

It is further understood that each range disclosed herein is to be interpreted as a disclosure of each specific value within the disclosed range that has the same number of significant digits. Thus, for example, a range from 1 to 4 is to be interpreted as an express disclosure of the values 1, 2, 3 and 10 4 as well as any range of such values.

It is further understood that each lower limit of each range disclosed herein is to be interpreted as disclosed in combination with each upper limit of each range and each specific value within each range disclosed herein for the same component, compounds, substituent or parameter. Thus, this disclosure to be interpreted as a disclosure of all ranges derived by combining each lower limit of each range with each upper limit of each range or with each specific value within each range, or by combining each upper limit of each range with each specific value within each range. That is, it is also further understood that any range between the endpoint values within the broad range is also discussed herein. Thus, a range from 1 to 4 also means a range from 1 to 3, 1 to 2, 2 to 4, 2 to 3, and so forth.

Furthermore, specific amounts/values of a component, compound, substituent or parameter disclosed in the description or an example is to be interpreted as a disclosure of either a lower or an upper limit of a range and thus can be combined with any other lower or upper limit of a range or specific amount/value for the same component, compound, substituent or parameter disclosed elsewhere in the application to form a range for that component, compound, substituent or parameter.

While particular embodiments have been described, alternatives, modifications, variations, improvements, and substantial equivalents that are or can be presently unforeseen can arise to applicants or others skilled in the art. Accordingly, the appended claims as filed and as they can be amended are intended to embrace all such alternatives, modifications variations, improvements, and substantial equivalents.

What is claimed is:

1. A low-ash lubricating oil composition suitable for use in lubricating the engine of a passenger car, the low-ash 45 lubricating oil composition including

one or more base oils of lubricating viscosity; a total calculated sulfated ash (SASH) of about 0.5 weight percent or less; about 0.02 to about 0.3 weight percent of an acyclic 50 corrosion inhibitor including one or more oil-soluble acids, diacids, acid-esters, or combinations thereof hav-

5

## 32

ing a C6 or greater hydrocarbyl chain and being substantially free of compounds having imine, imide, amidine structural units or hydroxy derivatives thereof, wherein the acyclic corrosion inhibitor is a blend of an oil-soluble diacid and an oil-soluble acid-ester each having the structure of Formula I:

(Formula I)



wherein

each of R<sub>1</sub> and R<sub>2</sub> is, independently, selected from —OH or —OR<sub>4</sub>OH with at least one of R<sub>1</sub> and R<sub>2</sub> being —OH; R<sub>3</sub> is a linear or branched C10 to C12 hydrocarbyl group; R<sub>4</sub> is a linear or branched C1 to C4 hydrocarbyl group with the —OH thereof being a primary or secondary alcohol;

wherein the lubricating oil composition is substantially free of a metal dialkyldithiophosphate; and

wherein the lubricating oil composition exhibits a stable emulsion at 0° C. and/or 25° C. pursuant to the E85 emulsion test of ASTM D7563 and no steel corrosion pursuant to the humidity corrosion test of GMW 16073.

2. The low-ash lubricating oil composition of claim 1, further comprising up to about 100 ppm of boron.

3. The low-ash lubricating oil composition of claim 1, wherein the lubricating oil composition is substantially free of a metallic detergent.

4. The low-ash lubricating oil composition of claim 3, wherein the lubricating oil composition has about 10 ppm or less of calcium, magnesium, or combinations thereof.

5. The low ash lubricating oil composition of claim 1, wherein the lubricating oil composition has about 10 ppm or less of zinc.

6. The low-ash lubricating oil composition of claim 1, wherein the lubricating oil composition further has about 30 mg or less of deposits when subjected to the high temperature deposit formation test of ASTM D6335.

7. The low-ash lubricating oil composition of claim 1, wherein the lubricating oil composition further has about 15 mg or less of deposits when subjected to the high temperature deposit formation test of ASTM D6335.

8. The low-ash lubricating oil composition of claim 1, wherein the lubricating oil composition is substantially free of corrosion inhibitors having aromatic moieties.

\* \* \* \* \*